



US008802191B2

(12) **United States Patent**  
**Zimmermann et al.**

(10) **Patent No.:** **US 8,802,191 B2**  
(45) **Date of Patent:** **\*Aug. 12, 2014**

(54) **METHOD FOR COATING A SUBSTRATE SURFACE AND COATED PRODUCT**

5,061,527 A 10/1991 Watanabe et al.  
5,091,244 A 2/1992 Biornard  
5,147,125 A 9/1992 Austin  
5,242,481 A 9/1993 Kumar  
5,270,858 A 12/1993 Dickey  
5,271,965 A 12/1993 Browning  
5,302,414 A 4/1994 Alkhimov et al.  
5,305,946 A 4/1994 Heilmann  
5,330,798 A 7/1994 Browning  
5,580,516 A 12/1996 Kumar  
5,612,254 A 3/1997 Mu et al.  
5,679,473 A 10/1997 Murayama et al.  
5,693,203 A 12/1997 Ohhashi et al.  
5,795,626 A 8/1998 Gabel et al.  
5,859,654 A 1/1999 Radke et al.  
5,954,856 A 9/1999 Pathare et al.  
5,972,065 A 10/1999 Dunn et al.  
5,993,513 A 11/1999 Fife  
6,030,577 A 2/2000 Commandeur et al.  
6,136,062 A 10/2000 Loffelholz et al.  
6,139,913 A 10/2000 Van Steenkiste et al.  
6,171,363 B1 1/2001 Shekhter et al.  
6,189,663 B1 2/2001 Smith et al.  
6,197,082 B1 3/2001 Dorvel et al.

(75) Inventors: **Stefan Zimmermann**, Laufenburg (DE); **Uwe Papp**, Harzburg (DE); **Heinrich Kreye**, Hamburg (DE); **Tobias Schmidt**, Eslohe (DE)

(73) Assignee: **H. C. Starck GmbH**, Goslar (DE)

(\*) Notice: Subject to any disclaimer, the term of this patent is extended or adjusted under 35 U.S.C. 154(b) by 1121 days.

This patent is subject to a terminal disclaimer.

(21) Appl. No.: **11/913,579**

(22) PCT Filed: **Apr. 28, 2006**

(86) PCT No.: **PCT/EP2006/003967**

§ 371 (c)(1),

(2), (4) Date: **Sep. 18, 2009**

(87) PCT Pub. No.: **WO2006/117144**

PCT Pub. Date: **Nov. 9, 2006**

(65) **Prior Publication Data**

US 2010/0055487 A1 Mar. 4, 2010

**Related U.S. Application Data**

(60) Provisional application No. 60/678,057, filed on May 5, 2005.

(51) **Int. Cl.**  
**B05D 1/12** (2006.01)

(52) **U.S. Cl.**  
USPC ..... **427/191**; 427/190; 427/192; 427/427;  
427/294

(58) **Field of Classification Search**

USPC ..... 427/190-192, 294, 427  
See application file for complete search history.

(56) **References Cited**

**U.S. PATENT DOCUMENTS**

3,436,299 A 4/1969 Halek  
3,990,784 A 11/1976 Gelber  
4,011,981 A 3/1977 Danna et al.  
4,073,427 A 2/1978 Keifert et al.  
4,140,172 A 2/1979 Corey  
4,202,932 A 5/1980 Chen et al.  
4,209,375 A 6/1980 Gates et al.  
4,291,104 A 9/1981 Keifert  
4,459,062 A 7/1984 Siebert  
4,483,819 A 11/1984 Albrecht et al.  
4,508,563 A 4/1985 Bernard et al.  
4,510,171 A 4/1985 Siebert  
4,537,641 A 8/1985 Albrecht et al.  
4,722,756 A 2/1988 Hard  
4,731,111 A 3/1988 Kopatz et al.  
4,818,629 A 4/1989 Jenstrom et al.  
4,915,745 A 4/1990 Pollock et al.  
4,964,906 A 10/1990 Fife

(Continued)

**FOREIGN PATENT DOCUMENTS**

|    |             |         |
|----|-------------|---------|
| CA | 2482287     | 10/2002 |
| DE | 10253794 A1 | 6/2004  |

(Continued)

**OTHER PUBLICATIONS**

“Cold Gas Dynamic Spray CGSM Apparatus,” Tev Tech LLC, available at: [http://www.tevtechllc.com/cold\\_gas.html](http://www.tevtechllc.com/cold_gas.html) (accessed Dec. 14, 2009). “Cold Spray Process,” Handbook of Thermal Spray Technology, ASM International, Sep. 2004, pp. 77-84.

Ajdelsztajn et al., “Synthesis and Mechanical Properties of Nanocrystalline Ni Coatings Produced by Cold Gas Dynamic Spraying,” 201 Surface and Coatings Tech. 3-4, pp. 1166-1172 (Oct. 2006). Examination Report in European Patent Application No. 09172234. 8, mailed Jun. 16, 2010 (3 pages).

Gärtner et al., “The Cold Spray Process and its Potential for Industrial Applications,” 15 J. of Thermal Sprays Tech. 2, pp. 223-232 (Jun. 2006).

Hall et al., “The Effect of a Simple Annealing Heat Treatment on the Mechanical Properties of Cold-Sprayed Aluminum,” 15 J. of Thermal Spray Tech. 2, pp. 233-238 (Jun. 2006.).

(Continued)

**Primary Examiner** — Frederick Parker

(74) **Attorney, Agent, or Firm** — Norman B. Thot

(57) **ABSTRACT**

Disclosed is a process for the reprocessing or production of a sputter target or an X-ray anode wherein a gas flow forms a gas/powder mixture with a powder of a material chosen from the group consisting of niobium, tantalum, tungsten, molybdenum, titanium, zirconium, mixtures of two or more thereof and alloys thereof with at least two thereof or with other metals, the powder has a particle size of 0.5 to 150  $\mu\text{m}$ , wherein a supersonic speed is imparted to the gas flow and the jet of supersonic speed is directed on to the surface of the object to be reprocessed or produced.

(56)

## References Cited

## U.S. PATENT DOCUMENTS

|                 |         |                       |                          |                  |                              |
|-----------------|---------|-----------------------|--------------------------|------------------|------------------------------|
| 6,238,456 B1    | 5/2001  | Wolf et al.           | 2004/0126499 A1          | 7/2004           | Heinrich et al.              |
| 6,245,390 B1    | 6/2001  | Baranovski et al.     | 2004/0202885 A1          | 10/2004          | Seth et al.                  |
| 6,258,402 B1    | 7/2001  | Hussary et al.        | 2005/0084701 A1          | 4/2005           | Slattery                     |
| 6,261,337 B1 *  | 7/2001  | Kumar .....           | 2005/0153069 A1 *        | 7/2005           | Tapphorn et al. .... 427/180 |
| 6,328,927 B1    | 12/2001 | Lo et al.             | 2005/0120957 A1          | 6/2005           | Kowalsky et al.              |
| 6,331,233 B1    | 12/2001 | Turner                | 2005/0142021 A1          | 6/2005           | Aimone et al.                |
| 6,408,928 B1    | 6/2002  | Heinrich et al.       | 2005/0147742 A1          | 7/2005           | Kleshock et al.              |
| 6,444,259 B1    | 9/2002  | Subramanian et al.    | 2005/0155856 A1          | 7/2005           | Oda                          |
| 6,464,933 B1    | 10/2002 | Popoola et al.        | 2005/0220995 A1          | 10/2005          | Hu et al.                    |
| 6,482,743 B1    | 11/2002 | Sato                  | 2005/0252450 A1          | 11/2005          | Kowalsky et al.              |
| 6,491,208 B2    | 12/2002 | James et al.          | 2006/0021870 A1          | 2/2006           | Tsai et al.                  |
| 6,502,767 B2    | 1/2003  | Kay et al.            | 2006/0027687 A1          | 2/2006           | Heinrich et al.              |
| 6,521,173 B2    | 2/2003  | Kumar et al.          | 2006/0032735 A1          | 2/2006           | Aimone et al.                |
| 6,558,447 B1    | 5/2003  | Shekhter et al.       | 2006/0042728 A1          | 3/2006           | Lemon et al.                 |
| 6,589,311 B1    | 7/2003  | Han et al.            | 2006/0045785 A1          | 3/2006           | Hu et al.                    |
| 6,623,796 B1    | 9/2003  | Van Steenkiste        | 2006/0090593 A1          | 5/2006           | Liu                          |
| 6,669,782 B1    | 12/2003 | Thakur                | 2006/0121187 A1 *        | 6/2006           | Haynes et al. .... 427/180   |
| 6,722,584 B2    | 4/2004  | Kay et al.            | 2006/0251872 A1          | 11/2006          | Wang et al.                  |
| 6,723,379 B2    | 4/2004  | Stark                 | 2007/0116886 A1          | 5/2007           | Refke et al.                 |
| 6,743,343 B2    | 6/2004  | Kida et al.           | 2007/0116890 A1          | 5/2007           | Adams et al.                 |
| 6,743,468 B2    | 6/2004  | Fuller et al.         | 2007/0172378 A1          | 7/2007           | Shibuya et al.               |
| 6,749,002 B2    | 6/2004  | Grinberg et al.       | 2007/0183919 A1          | 8/2007           | Ayer et al.                  |
| 6,759,085 B2    | 7/2004  | Muehlberger           | 2007/0187525 A1 *        | 8/2007           | Jabado et al. .... 239/79    |
| 6,770,154 B2    | 8/2004  | Koenigsmann et al.    | 2007/0196570 A1          | 8/2007           | Gentsch et al.               |
| 6,773,969 B2    | 8/2004  | Lee et al.            | 2008/0028459 A1          | 1/2008           | Suh et al.                   |
| 6,780,458 B2    | 8/2004  | Seth et al.           | 2008/0078268 A1          | 4/2008           | Shekhter et al.              |
| 6,855,236 B2    | 2/2005  | Sato et al.           | 2008/0145688 A1          | 6/2008           | Miller et al.                |
| 6,872,425 B2    | 3/2005  | Kaufold et al.        | 2008/0171215 A1          | 7/2008           | Kumar et al.                 |
| 6,872,427 B2    | 3/2005  | Van Steenkiste et al. | 2008/0216602 A1          | 9/2008           | Zimmermann et al.            |
| 6,896,933 B2    | 5/2005  | Van Steenkiste et al. | 2008/0271779 A1          | 11/2008          | Miller et al.                |
| 6,905,728 B1    | 6/2005  | Hu et al.             | 2009/0004379 A1          | 1/2009           | Deng et al.                  |
| 6,911,124 B2    | 6/2005  | Tang et al.           | 2009/0239754 A1          | 9/2009           | Kruger et al.                |
| 6,915,964 B2    | 7/2005  | Tapphorn et al.       | 2009/0291851 A1          | 11/2009          | Bohn et al.                  |
| 6,919,275 B2    | 7/2005  | Chiang et al.         | 2010/0015467 A1          | 1/2010           | Zimmermann et al.            |
| 6,924,974 B2    | 8/2005  | Stark                 | 2010/0061876 A1          | 3/2010           | Miller et al.                |
| 6,953,742 B2    | 10/2005 | Chen et al.           | 2010/0084052 A1          | 4/2010           | Farmer et al.                |
| 6,962,407 B2    | 11/2005 | Yamamoto et al.       | 2010/0086800 A1          | 4/2010           | Miller et al.                |
| 7,053,294 B2    | 5/2006  | Tuttle et al.         | 2010/0136242 A1          | 6/2010           | Kay et al.                   |
| 7,067,197 B2    | 6/2006  | Michaluk et al.       | 2010/0172789 A1          | 7/2010           | Calla et al.                 |
| 7,081,148 B2    | 7/2006  | Koenigsmann et al.    | 2010/0189910 A1          | 7/2010           | Belashchenko et al.          |
| 7,101,447 B2    | 9/2006  | Turner                | 2010/0246774 A1          | 9/2010           | Lathrop                      |
| 7,108,893 B2    | 9/2006  | Van Steenkiste et al. | 2010/0272889 A1          | 10/2010          | Shekhter et al.              |
| 7,128,988 B2    | 10/2006 | Lambeth               | 2011/0132534 A1          | 6/2011           | Miller et al.                |
| 7,143,967 B2    | 12/2006 | Heinrich et al.       | 2011/0300396 A1          | 12/2011          | Miller et al.                |
| 7,163,715 B1    | 1/2007  | Kramer                | 2011/0303535 A1          | 12/2011          | Miller et al.                |
| 7,164,205 B2    | 1/2007  | Yamaji et al.         | FOREIGN PATENT DOCUMENTS |                  |                              |
| 7,170,915 B2    | 1/2007  | McDonald              | EP                       | 0074803 A1       | 3/1983                       |
| 7,175,802 B2    | 2/2007  | Sandlin et al.        | EP                       | 0484533 A1       | 5/1992                       |
| 7,178,744 B2    | 2/2007  | Tapphorn et al.       | EP                       | 0774315 A2       | 5/1997                       |
| 7,183,206 B2    | 2/2007  | Shepard               | EP                       | 1066899 A2       | 1/2001                       |
| 7,192,623 B2    | 3/2007  | Andre et al.          | EP                       | 1138420 A2       | 10/2001                      |
| 7,208,230 B2    | 4/2007  | Ackerman et al.       | EP                       | 1350861 A1       | 10/2003                      |
| 7,244,466 B2    | 7/2007  | Van Steenkiste et al. | EP                       | 1382720 A2       | 1/2004                       |
| 7,278,353 B2    | 10/2007 | Langan et al.         | EP                       | 1398394          | 3/2004                       |
| 7,335,341 B2    | 2/2008  | Van Steenkiste et al. | EP                       | 1413642 A1       | 4/2004                       |
| 7,399,335 B2    | 7/2008  | Shekhter et al.       | EP                       | 1452622          | 9/2004                       |
| 7,402,277 B2    | 7/2008  | Ayer et al.           | EP                       | 1715080          | 10/2006                      |
| 7,479,299 B2    | 1/2009  | Raybould et al.       | GB                       | 2121441 A        | 12/1983                      |
| 7,514,122 B2    | 4/2009  | Kramer                | GB                       | 2394479 A        | 4/2004                       |
| 7,582,846 B2    | 9/2009  | Molz et al.           | JP                       | 54067198         | 5/1979                       |
| 7,618,500 B2    | 11/2009 | Farmer et al.         | JP                       | 3197640          | 8/1991                       |
| 7,670,406 B2    | 3/2010  | Belashchenko          | JP                       | 06346232 A       | 12/1994                      |
| 7,910,051 B2    | 3/2011  | Zimmermann et al.     | JP                       | 11269639         | 10/1999                      |
| 8,002,169 B2    | 8/2011  | Miller et al.         | JP                       | 11-312484 A      | 11/1999                      |
| 8,043,655 B2    | 10/2011 | Miller et al.         | JP                       | 01/131767        | 5/2001                       |
| 2001/0014568 A1 | 8/2001  | Itoh et al.           | JP                       | 03/301278        | 10/2003                      |
| 2002/0112789 A1 | 8/2002  | Jepson et al.         | JP                       | 2004-307969 A    | 11/2004                      |
| 2002/0112955 A1 | 8/2002  | Aimone et al.         | JP                       | 2005-29858 A     | 2/2005                       |
| 2003/0023132 A1 | 1/2003  | Melvin et al.         | JP                       | 2005-95886 A     | 4/2005                       |
| 2003/0190413 A1 | 10/2003 | Van Steenkiste et al. | RU                       | 2166421 C1       | 5/2001                       |
| 2003/0219542 A1 | 11/2003 | Ewasysyhn et al.      | WO                       | WO-98/37249 A1   | 8/1998                       |
| 2003/0232132 A1 | 12/2003 | Muehlberger           | WO                       | WO-01/12364 A1   | 2/2001                       |
| 2004/0037954 A1 | 2/2004  | Heinrich et al.       | WO                       | WO-02/064287 A2  | 8/2002                       |
| 2004/0065546 A1 | 4/2004  | Michaluk et al.       | WO                       | WO-02/070765     | 9/2002                       |
| 2004/0076807 A1 | 4/2004  | Grinberg et al.       | WO                       | WO-03062491 A2   | 7/2003                       |
|                 |         |                       | WO                       | WO-03106051 A1   | 12/2003                      |
|                 |         |                       | WO                       | WO-2004074540 A1 | 9/2004                       |

(56)

**References Cited**

## FOREIGN PATENT DOCUMENTS

|    |                |    |         |
|----|----------------|----|---------|
| WO | WO-2005073418  | A1 | 8/2005  |
| WO | WO-2005/079209 |    | 9/2005  |
| WO | WO-2006/117145 |    | 11/2006 |
| WO | WO 2006/117145 |    | 11/2006 |
| WO | WO-2007/001441 |    | 1/2007  |
| WO | WO-2008/063891 |    | 5/2008  |
| WO | WO-2008/089188 | A1 | 7/2008  |

## OTHER PUBLICATIONS

- Hall et al., "Preparation of Aluminum Coatings Containing Homogeneous Nanocrystalline Microstructures Using the Cold Spray Process," *JTTEES* 17:352-359.
- IPRP in International Patent Application No. PCT/EP2006/003967, dated Nov. 6, 2007 (15 pages).
- IPRP in International Patent Application No. PCT/US2008/062434, dated Nov. 10, 2009 (21 pages).
- IPRP in International Patent Application No. PCT/EP2006/003969, mailed dated Nov. 6, 2007 (13 pages).
- International Search Report and Written Opinion in International Patent Application No. PCT/US2007/087214, mailed Mar. 23, 2009 (13 pages).
- IPRP in International Patent Application No. PCT/US2007/081200, dated Sep. 1, 2009 (17 pages).
- IPRP in International Patent Application No. PCT/US2007/080282, dated Apr. 7, 2009 (15 pages).
- Irisso et al., "Review on Cold Spray Process and Technology: Part I—Intellectual Property," *17 J. of Thermal Spray Tech.* 4, pp. 495-516 (Dec. 2008).

Karthikeyan, "Cold Spray Technology: International Status and USA Efforts," ASB Industries, Inc. (Dec. 2004).

Li et al., "Effect of Annealing Treatment on the Microstructure and Properties of Cold-Sprayed Cu Coating," *15 J. of Thermal Spray Tech.* 2, pp. 206-211 (Jun. 2006).

Marx et al., "Cold Spraying—Innovative Layers for New Applications," *15 J. of Thermal Spray Tech.* 2, pp. 177-183 (Jun. 2006).

Morito, "Preparation and Characterization of Sintered Mo—Re Alloys," *3 J. de Physique* 7, Part 1, pp. 553-556 (1993).

Search Report in European Patent Application No. 09172234.8, dated Jan. 29, 2010 (7 pages).

Stoltenhoff et al., "An Analysis of the Cold Spray Process and its Coatings," *11 J. of Thermal Spray Tech.* 4, pp. 542-550 (Dec. 2002).

Van Steenkiste et al., "Analysis of Tantalum Coatings Produced by the Kinetic Spray Process," *13 J. of Thermal Spray Tech.* 2, pp. 265-273 (Jun. 2004).

Kosarev et al., "Recently Patent Facilities and Applications in Cold Spray Engineering," *Recent Patents on Engineering*, vol. 1 pp. 35-42 (2007).

Examination Report in European Patent Application No. 07843733.2, mailed Nov. 30, 2010 (9 pages).

English Translation of Office Action mailed Feb. 23, 2011 for Chinese Patent Application No. 200880023411.5 (7 pages).

Examination Report in European Patent Application No. 08755010.9, mailed Sep. 16, 2011 (3 pages).

Examination Report in Canadian Patent Application No. 2,736,876, mailed Feb. 29, 2012 (4 pages).

Tapphorn et al., "The Solid-State Spray Forming of Low-Oxide Titanium Components," *JOM*, p. 45-47 (1998).

\* cited by examiner



**Fig. 1**



**Fig. 2**



**Fig. 3**



**Fig. 4**



**Fig. 5**



**Fig. 6**



**Fig. 7**



**Fig. 8**



Fig. 9



Fig. 10

## 1

METHOD FOR COATING A SUBSTRATE  
SURFACE AND COATED PRODUCTCROSS-REFERENCE TO RELATED  
APPLICATIONS

This application is a national stage application, under 35 U.S.C. §371, of PCT/EP2006/003967, filed Apr. 28, 2005, which claims priority to U.S. Provisional Application No. 60/678,057, filed May 5, 2005.

## BACKGROUND OF THE INVENTION

The present invention relates to a method of applying coatings which contain only small amounts of gaseous impurities, in particular oxygen.

The application of refractory metal coatings to surfaces exhibits numerous problems.

In conventional processes, the metal is completely or partially melted in most cases, as a result of which the metals readily oxidise or absorb other gaseous impurities. For this reason, conventional processes such as deposition-welding and plasma spraying must be carried out under a protecting gas or in vacuo.

In such cases, the outlay in terms of apparatus is high, the size of the components is limited, and the content of gaseous impurities is still unsatisfactory.

The pronounced introduction of heat transmitted into the object to be coated leads to a very high potential for distortion and means that these processes cannot be employed in the case of complex components, which often also contain constituents that melt at low temperatures. Complex components must therefore be taken apart before they are re-processed, with the result, in general, that re-processing is scarcely economical and only recycling of the material of the components (scrapping) is carried out.

Moreover, in the case of vacuum plasma spraying, tungsten and copper impurities, which originate from the electrodes used, are introduced into the coating, which is generally undesirable. In the case of, for example, the use of tantalum or niobium coatings for corrosion protection, such impurities reduce the protective effect of the coating by the formation of so-called micro-galvanic cells.

Moreover, such processes are processes of melt metallurgy, which always involve the inherent disadvantages thereof, such as, for example, unidirectional grain growth. This occurs in particular in laser processes, where a suitable powder is applied to the surface and melted by means of a laser beam. A further problem is the porosity, which can be observed in particular when a metal powder is first applied and is subsequently melted by means of a heat source. Attempts have been made in WO 02/064287 to solve these problems by merely melting on the powder particles by means of an energy beam, such as, for example, laser beams, and sintering them. However, the results are not always satisfactory and a high outlay in terms of apparatus is required, and the problems associated with the introduction of a reduced but nevertheless high amount of energy into a complex component remain.

WO-A-03/106,051 discloses a method and an apparatus for low pressure cold spraying. In this process a coating of powder particles is sprayed in a gas substantially at ambient temperatures onto a workpiece. The process is conducted in a low ambient pressure environment which is less than atmospheric pressure to accelerate the sprayed powder particles. With this process a coating of a powder is formed on a workpiece.

## 2

EP-A-1,382,720 discloses another method and apparatus for low pressure cold spraying. In this process the target to be coated and the cold spray gun are located within a vacuum chamber at pressures below 80 kPa. With this process a workpiece is coated with a powder.

## BRIEF SUMMARY OF THE INVENTION

In view of this prior art it was therefore the object, to provide a novel process for coating substrates which is distinguished by the introduction of a small amount of energy, a low outlay in terms of apparatus and broad applicability for different carrier materials and coating materials, and wherein the metal to be applied is not melted on during processing.

Another object of this invention was the provision of a novel process for preparing dense and corrosion resistant coatings, especially tantalum coatings, which possess low content of impurities, preferably low content of oxygen and nitrogen impurities, which coatings are highly qualified for use as corrosion protective layer, especially in equipment of chemical plants.

The object of the present invention is achieved by applying a desired refractory metal to the desired surface by a method as claimed in claim 1.

There are generally suitable for this purpose processes in which, in contrast to the conventional processes of thermal spraying (flame, plasma, high-velocity flame, arc, vacuum plasma, low-pressure plasma spraying) and of deposition-welding, there is no melting on of the coating material, caused by thermal energy produced in the coating apparatus. Contact with a flame or hot combustion gases is to be avoided, because these can cause oxidation of the powder particles and hence the oxygen content in the resulting coatings rises.

These processes are known to the person skilled in the art as, for example, cold gas spraying, cold spray processes, cold gas dynamic spraying, kinetic spraying and are described, for example, in EP-A-484533. Also suitable according to the invention is the process described in patent DE-A-10253794.

The so-called cold spray process or the kinetic spray process are particularly suitable for the method according to the invention; the cold spray process, which is described in EP-A-484533, is especially suitable, and this specification is incorporated herein by reference.

## A BRIEF DESCRIPTION OF THE FIGURES

FIG. 1: Unetched cross-section of a tantalum coating, process gas helium.

FIG. 2: Unetched cross-section of a tantalum coating, process gas helium, overview picture with low magnification.

FIG. 3: Cross-section of a tantalum coating, etched with hydrofluoric acid, process gas helium, overview picture with low magnification.

FIG. 4: Cross-section of a tantalum coating, etched with hydrofluoric acid, process gas helium.

FIG. 5: Image section used for porosity determination, cross-section of a tantalum coating, process gas helium.

FIG. 6: Cross-section of a tantalum coating, etched with hydrofluoric acid, interface with the substrate, process gas helium.

FIG. 7: Unetched cross-section of a tantalum coating, process gas nitrogen, overview picture with low magnification.

FIG. 8: Unetched cross-section of a tantalum coating, process gas nitrogen.

FIG. 9: Image section used for porosity determination, cross-section of a tantalum coating, process gas nitrogen.

FIG. 10: Unetched cross-section of a tantalum coating, process gas nitrogen, high magnification.

#### DETAILED DESCRIPTION OF THE INVENTION

Accordingly, there is advantageously employed a method for applying coatings to surfaces, wherein a gas flow forms a gas-powder mixture with a powder of a material selected from the group consisting of niobium, tantalum, tungsten, molybdenum, titanium, zirconium, mixtures of at least two thereof or their alloys with one another or with other metals, the powder has a particle size of from 0.5 to 150  $\mu\text{m}$ , wherein a supersonic speed is imparted to the gas flow and a jet of supersonic speed is formed, which ensures a speed of the powder in the gas-powder mixture of from 300 to 2000 m/s, preferably from 300 to 1200 m/s, and the jet is directed onto the surface of an object.

The metal powder particles striking the surface of the object form a coating, the particles being deformed very considerably.

The powder particles are advantageously present in the jet in an amount that ensures a flow rate density of the particles of from 0.01 to 200 g/s  $\text{cm}^2$ , preferably 0.01 to 100 g/s  $\text{cm}^2$ , very preferably 0.01 g/s  $\text{cm}^2$  to 20 g/s  $\text{cm}^2$ , or most preferred from 0.05 g/s  $\text{cm}^2$  to 17 g/s  $\text{cm}^2$ .

The flow rate density is calculated according to the formula  $F=m/(\pi/4*D^2)$  where  $F$ =flow rate density,  $D$ =nozzle cross-section,  $m$ =powder feed rate. A powder feed rate of, for example, 70 g/min=1.1667 g/s is a typical example of a powder feed rate.

At low  $D$  values of below 2 mm values of markedly greater than 20 g/s  $\text{cm}^2$  can be achieved. In this case  $F$  can easily assume values 50 g/s  $\text{cm}^2$  or even higher at higher powder delivery rates.

As the gas with which the metal powder forms a gas-powder mixture there is generally used an inert gas such as argon, neon, helium, nitrogen or mixtures of two or more thereof. In particular cases, air may also be used. If safety regulations are met also use of hydrogen or mixtures of hydrogen with other gases can be used.

In a preferred version of the process the spraying comprises the steps of:

providing a spraying orifice adjacent a surface to be coated by spraying;

providing to the spraying orifice a powder of a particulate material chosen from the group consisting of niobium, tantalum, tungsten, molybdenum, titanium, zirconium, mixtures of at least two thereof or alloys thereof with one another or other metals, the powder having a particle size of 0.5 to 150  $\mu\text{m}$ , said powder being under pressure;

providing an inert gas under pressure to the spraying orifice to establish a static pressure at the spraying orifice and providing a spray of said particulate material and gas onto the surface to be coated; and

locating the spraying orifice in a region of low ambient pressure which is less than 1 atmosphere and which is substantially less than the static pressure at the spraying orifice to provide substantial acceleration of the spray of said particulate material and gas onto said surface to be coated.

In another preferred version of the process the spraying is performed with a cold spray gun and the target to be coated and the cold spray gun are located within a vacuum chamber at pressures below 80 kPa, preferably between 0.1 and 50 kPa,

and most preferred between 2 and 10 kPa. Further advantageous embodiments can be found in the claims.

In general, the refractory metal has a purity of 99% or more, such as 99.5% or 99.7% or 99.9%.

5 According to the invention, the refractory metal advantageously has a purity of at least 99.95%, based on metallic impurities, especially of at least 99.995% or of at least 99.999%, in particular of at least 99.9995%. If an alloy is used instead of a single refractory metal, then at least the refractory metal, but preferably the alloy as a whole, has that purity, so that a corresponding highly pure coating can be produced.

In addition, the metal powder has an oxygen content of less than 1000 ppm oxygen, or less than 500, or less than 300, in particular an oxygen content of less than 100 ppm.

15 Particularly suitable refractory metal powders have a purity of at least 99.7%, advantageously of at least 99.9%, in particular 99.95%, and a content of less than 1000 ppm oxygen, or less than 500 ppm oxygen, or less than 300 ppm oxygen, in particular an oxygen content of less than 100 ppm.

20 Particularly suitable refractory metal powders have a purity of at least 99.95%, in particular of at least 99.995%, and a content of less than 1000 ppm oxygen, or less than 500 ppm oxygen, or less than 300 ppm oxygen, in particular an oxygen content of less than 100 ppm.

25 Particularly suitable refractory metal powders have a purity of at least 99.999%, in particular of at least 99.995%, and a content of less than 1000 ppm oxygen, or less than 500 ppm oxygen, or less than 300 ppm oxygen, in particular an oxygen content of less than 100 ppm.

30 In all the above-mentioned powders, the total content of other non-metallic impurities, such as carbon, nitrogen or hydrogen, should advantageously be less than 500 ppm, preferably less than 150 ppm.

35 In particular, the oxygen content is advantageously 50 ppm or less, the nitrogen content is 25 ppm or less and the carbon content is 25 ppm or less.

The content of metallic impurities is advantageously 500 ppm or less, preferably 100 ppm or less and most preferably 50 ppm or less, in particular 10 ppm or less.

40 Suitable metal powders are, for example, many of the refractory metal powders which are also suitable for the production of capacitors.

45 Such metal powders can be prepared by reduction of refractory metal compound with a reducing agent and preferably subsequent deoxidation. Tungsten oxide or molybdenum oxide, for example, is reduced in a stream of hydrogen at elevated temperature. The preparation is described, for example, in Schubert, Lassner, "Tungsten", Kluwer Academic/Plenum Publishers, New York, 1999 or Brauer, "Handbuch der Präparativen Anorganischen Chemie", Ferdinand Enke Verlag Stuttgart, 1981, p 1530.

50 In the case of tantalum and niobium, the preparation is in most cases carried out by reducing alkali heptafluoro-tantalates and earth alkaline metal heptafluoro-tantalates or the oxides, such as, for example, sodium heptafluorotantalate, potassium heptafluorotantalate, sodium heptafluoroniobate or potassium heptafluoroniobate, with an alkali or alkaline earth metal. The reduction can be carried out in a salt melt with the addition of, for example, sodium, or in the gas phase, calcium or magnesium vapour advantageously being used. It is also possible to mix the refractory metal compound with the alkali or alkaline earth metal and heat the mixture. A hydrogen atmosphere may be advantageous. A large number of suitable processes is known to the person skilled in the art, as 55 are process parameters from which suitable reaction conditions can be selected. Suitable processes are described, for example, in U.S. Pat. No. 4,483,819 and WO 98/37249.

After the reduction, deoxidation is preferably carried out. This can be effected, for example, by mixing the refractory metal powder with Mg, Ca, Ba, La, Y or Ce and then heating, or by heating the refractory metal in the presence of a getter in an atmosphere that allows oxygen to pass from the metal powder to the getter. The refractory metal powder is in most cases then freed of the salts of the deoxidising agent using an acid and water, and is dried.

It is advantageous if, when using metals to lower the oxygen content, the metallic impurities can be kept low. A further process for preparing pure powder having a low oxygen content consists in reducing a refractory metal hydride using an alkaline earth metal as reducing agent, as disclosed, for example, in WO 01/12364 and EP-A-1200218.

The thickness of the coating is usually more than 0.01 mm. Preferred are layers with a thickness between 0.05 and 10 mm, more preferred between 0.05 and 5 mm, still more preferred between 0.05 and 1 mm, still more preferred between 0.05 and 0.5 mm. The thickness may be higher as well, for example from 3 to 50 mm, or from 5 to 45 mm, or from 8 to 40 mm, or from 10 to 30 mm or from 10 to 20 mm or 10 to 15 mm.

The purities and oxygen contents of the resulting coatings should deviate not more than 50% and preferably not more than 20% from those of the powder.

Advantageously, this can be achieved by coating the substrate surface under an inert gas. Argon is advantageously used as the inert gas because, owing to its higher density than air, it tends to cover the object to be coated and to remain present, in particular when the surface to be coated is located in a vessel which prevents the argon from escaping or flowing away and more argon is continuously added.

The coatings applied according to the invention have a high purity and a low oxygen content. Advantageously, these coatings have an oxygen content of less than 1000 ppm oxygen, or less than 500, or less than 300, in particular an oxygen content of less than 100 ppm.

The coatings usually exhibit compressive stress  $\sigma$ . Usually, the compressive stress is about -1000 MPa to 0 MPa, or from -700 MPa to 0 MPa, or from -500 MPa to 0 MPa, or from -400 MPa to 0 MPa or from -300 MPa to 0. More specifically, the compressive stress is from -200 MPa to -1000 MPa, or from -300 MPa to -700 MPa, or from -300 MPa to -500 MPa.

In general, a lower oxygen content of the powder employed will result in layers exhibiting lower compressive stress, e.g. a layer sprayed from powder having an oxygen content of 1400 ppm will usually result in a layer exhibiting compressive stress of about  $-970 \pm 50$  MPa and a layer sprayed from powder having an oxygen content of 270 ppm will usually result in a layer exhibiting compressive stress of about  $-460 \text{ MPa} \pm 50 \text{ MPa}$ , more preferably  $-400 \text{ MPa} \pm 50 \text{ MPa}$ .

In contrast thereto, layers produced by plasma spraying result in layers exhibiting no compressive stress at all, but tensile stress.

In particular, these coatings have a purity of at least 99.7%, advantageously of at least 99.9%, in particular of at least 99.95%, and a content of less than 1000 ppm oxygen, or less than 500 ppm oxygen, or less than 300 ppm oxygen, in particular an oxygen content of less than 100 ppm.

In particular, these coatings have a purity of at least 99.95%, in particular of at least 99.995%, and a content of less than 1000 ppm oxygen, or less than 500 ppm oxygen, or less than 300 ppm oxygen, in particular an oxygen content of less than 100 ppm.

In particular, these coatings have a purity of 99.999%, in particular of at least 99.9995%, and a content of less than

1000 ppm oxygen, or less than 500 ppm oxygen, or less than 300 ppm oxygen, in particular an oxygen content of less than 100 ppm.

The coatings according to the invention have a total content of other non-metallic impurities, such as carbon, nitrogen or hydrogen, which is advantageously below 500 ppm and most preferably below 150 ppm.

The applied coating has a content of gaseous impurities which differs by not more than 50%, or not more than 20%, or not more than 10%, or not more than 5%, or not more than 1%, from the content of the starting powder with which this coating was produced. The term "differs" is to be understood as meaning in particular an increase; the resulting coatings should, therefore, advantageously have a content of gaseous impurities that is not more than 50% greater than the content of the starting powder.

The applied coating preferably has an oxygen content which differs by not more than 5%, in particular not more than 1%, from the oxygen content of the starting powder.

The coatings according to the invention preferably have a total content of other non-metallic impurities, such as carbon, nitrogen or hydrogen, which is advantageously less than 500 ppm and most preferably less than 150 ppm. With the process of this invention layers with higher impurity contents can also be produced.

In particular, the oxygen content is advantageously 50 ppm or less, the nitrogen content is 25 ppm or less and the carbon content is 25 ppm or less.

The content of metallic impurities is advantageously 50 ppm or less, in particular 10 ppm or less.

In an advantageous embodiment, the coatings additionally have a density of at least 97%, preferably greater than 98%, in particular greater than 99% or 99.5%. 97% density of a layer means that the layer has a density of 97% of the bulk material. The density of the coating is here a measure of the closed nature and porosity of the coating. A closed, substantially pore-free coating always has a density of more than 99.5%. The density can be determined either by image analysis of a cross-sectional image (ground section) of such a coating, or alternatively by helium pycnometry. The latter method is less preferred because, in the case of very dense coatings, pores present in coatings that are more remote from the surface are not detected and a lower porosity is accordingly measured than actually exists. By means of image analysis, the density can be determined by first determining the total area of the coating to be investigated in the image area of the microscope and relating this area to the areas of the pores. In this method, pores that are located far from the surface and close to the interface with the substrate are also detected. A high density of at least 97%, preferably greater than 98%, in particular greater than 99% or 99.5%, is important in many coating processes.

The coatings show high mechanical strength which is caused by their high density and by the high deformation of the particles. In the case of tantalum, therefore, the strengths are at least 80 MPa more preferably at least 100 MPa, most preferably at least 140 MPa when nitrogen is used as the gas with which the metal powder forms a gas-powder mixture. If helium is used, the strength usually is at least 150 MPa, preferably at least 170 MPa, most preferably at least 200 MPa and very most preferred greater than 250 MPa.

Although the coatings according to the invention show high densities and low porosities, the coatings have a morphology clearly showing it was created from discrete particles. Examples can be seen, for example, in FIGS. 1 to 7. In this way the coatings according to the invention can be distinguished over coatings obtained by other methods, like

coatings obtained by galvanic processes. The characteristic appearance also allows distinguishing of coatings according to the invention from coatings obtained by plasma spraying.

The articles to be coated with the process of this invention are not limited. Generally all articles which need a coating, preferably a corrosion protective coating, can be used. These articles may be made of metal and/or of ceramic material and/or of plastic material or may comprise components from these materials. Preferably surfaces of materials are coated which are subject to removal of material, for example by wear, corrosion, oxidation, etching, machining or other stress.

Preferably surfaces of materials are coated with the process of this invention which are used in corroding surroundings, for example in chemical processes in medical devices or in implants. Examples of apparatus or components to be coated are components used in chemical plants or in laboratories or in medical devices or as implants, such as reaction and mixing vessels, stirrers, blind flanges, thermowells, bursting disks, bursting disk holders, heat exchangers (shell and tubes), pipings, valves, valve bodies and pump parts.

Preferably articles are coated with the process of this invention which are no sputter targets or X-ray anodes.

The coatings prepared with the process of this invention preferably are used in corrosion protection.

The present invention therefore relates also to articles made of metal and/or of ceramic material and/or of plastic material containing at least one coatings composed of the refractory metals niobium, tantalum, tungsten, molybdenum, titanium, zirconium or mixtures of two or more thereof or alloys of two or more thereof or alloys with other metals, which coatings have the above-mentioned properties.

Such coatings are in particular coatings of tantalum or niobium.

Preferably layers of tungsten, molybdenum, titanium zirconium or mixtures of two or more thereof or alloys of two or more thereof or alloys with other metals, very preferably layers of tantalum or niobium, are applied by cold spraying to the surface of a substrate to be coated. Surprisingly it has been found that with said powders or powder mixtures, preferably with tantalum and niobium powders, possessing a reduced oxygen content, for example an oxygen content below 1000 ppm, there can be produced cold sprayed layers with very high deposition rates of more than 90%. In said cold sprayed layers the oxygen content of the metal is nearly unchanged compared to the oxygen content of the powders. These cold sprayed layers show considerably higher densities than layers produced by plasma spraying or by vacuum spraying. Furthermore, these cold sprayed layers can be produced without any or with small texture, depending on powder properties and coating parameters. These cold sprayed layers are also object of this invention.

Suitable metal powders for use in the methods according to the invention are also metal powders that consist of alloys, pseudo alloys and powder mixtures of refractory metals with suitable non-refractory metals.

It is thereby possible to coat surfaces of substrates made of the same alloy or pseudo alloy.

These include especially alloys, pseudo alloys or powder mixtures of a refractory metal selected from the group consisting of niobium, tantalum, tungsten, molybdenum, titanium, zirconium or mixtures of two or more thereof, with a metal selected from the group cobalt, nickel, rhodium, palladium, platinum, copper, silver and gold. Such powders belong to the prior art, are known in principle to the person skilled in the art and are described, for example, in EP-A-774315 and EP-A-1138420.

They can be prepared by conventional processes; for example, powder mixtures are obtainable by homogenously mixing pre-prepared metal powders, it being possible for the mixing to be carried out on the one hand before use in the method according to the invention or alternatively during production of the gas-powder mixture. Alloy powders are in most cases obtainable by melting and mixing the alloying partners. According to the invention there may be used as alloy powders also so-called pre-alloyed powders. These are powders which are produced by mixing compounds such as, for example, salts, oxides and/or hydrides of the alloying partners and then reducing them, so that intimate mixtures of the metals in question are obtained. It is additionally possible according to the invention to use pseudo alloys. Pseudo alloys are understood as being materials which are obtained not by conventional melt metallurgy but, for example, by grinding, sintering or infiltration.

Known materials are, for example, tungsten/copper alloys or tungsten/copper mixtures, the properties of which are known and are listed here by way of example:

| Type  | Density<br>(g/cm <sup>3</sup> ) | HB (MPa) | Electrical<br>conductivity<br>(% IACS) | Thermal<br>expansion<br>coefficient<br>(ppm/K) | Thermal<br>conductivity<br>(W/m · K) |
|-------|---------------------------------|----------|----------------------------------------|------------------------------------------------|--------------------------------------|
|       |                                 |          |                                        | (ppm/K)                                        | (W/m · K)                            |
| WCu10 | 16.8-17.2                       | ≥2550    | >27                                    | 6.5                                            | 170-180                              |
| WCu15 | 16.3                            |          |                                        | 7.0                                            | 190-200                              |
| WCu20 | 15.2-15.6                       | ≥2160    | >34                                    | 8.3                                            | 200-220                              |
| WCu25 | 14.5-15.0                       | ≥1940    | >38                                    | 9.0                                            | 220-250                              |
| WCu30 | 13.8-14.4                       | ≥1720    | >42                                    |                                                |                                      |

Also known are molybdenum-copper alloys or molybdenum/copper mixtures in the same ratios as indicated above.

Also known are molybdenum-silver alloys or molybdenum/silver mixtures which contain, for example, 10, 40 or 65 wt. % molybdenum.

Also known are tungsten-silver alloys or tungsten/silver mixtures which contain, for example, 10, 40 or 65 wt. % tungsten.

These can be used, for example, in heat pipes, cooling bodies or, in general, in temperature management systems.

It is also possible to use tungsten-rhenium alloys or mixtures, or the metal powder is an alloy having the following composition:

from 94 to 99 wt. %, preferably from 95 to 97 wt. %, molybdenum, from 1 to 6 wt. %, preferably from 2 to 4 wt. %, niobium, from 0.05 to 1 wt. %, preferably from 0.05 to 0.02 wt. %, zirconium.

These alloys, like pure refractory metal powders having a purity of at least 99.95%, can be used in the recycling or production of sputter targets by means of cold gas spraying.

Suitable materials for the methods according to the invention are listed in Tables 1 to 15. Individual materials are designated with the number of the table followed by the number of the combination of components and the amount of the non-refractory metal as in Table 1. For example, material 2.005 is a material described in Table 2, the precise composition being defined with the non-refractory metal and the amount thereof as listed in Table 1, position no. 5.

Suitable niobium alloys are listed in Table 1.

TABLE 1

| No.   | Refractory metal | Non-refractory metal | Amount of non-refractory metal (wt. %) |
|-------|------------------|----------------------|----------------------------------------|
| 1.001 | Niobium          | Cobalt               | 2-5                                    |
| 1.002 | Niobium          | Nickel               | 2-5                                    |
| 1.003 | Niobium          | Rhodium              | 2-5                                    |
| 1.004 | Niobium          | Palladium            | 2-5                                    |
| 1.005 | Niobium          | Platinum             | 2-5                                    |
| 1.006 | Niobium          | Copper               | 2-5                                    |
| 1.007 | Niobium          | Silver               | 2-5                                    |
| 1.008 | Niobium          | Gold                 | 2-5                                    |
| 1.009 | Niobium          | Cobalt               | 5-10                                   |
| 1.010 | Niobium          | Nickel               | 5-10                                   |
| 1.011 | Niobium          | Rhodium              | 5-10                                   |
| 1.012 | Niobium          | Palladium            | 5-10                                   |
| 1.013 | Niobium          | Platinum             | 5-10                                   |
| 1.014 | Niobium          | Copper               | 5-10                                   |
| 1.015 | Niobium          | Silver               | 5-10                                   |
| 1.016 | Niobium          | Gold                 | 5-10                                   |
| 1.017 | Niobium          | Cobalt               | 10-15                                  |
| 1.018 | Niobium          | Nickel               | 10-15                                  |
| 1.019 | Niobium          | Rhodium              | 10-15                                  |
| 1.020 | Niobium          | Palladium            | 10-15                                  |
| 1.021 | Niobium          | Platinum             | 10-15                                  |
| 1.022 | Niobium          | Copper               | 10-15                                  |
| 1.023 | Niobium          | Silver               | 10-15                                  |
| 1.024 | Niobium          | Gold                 | 10-15                                  |
| 1.025 | Niobium          | Cobalt               | 15-20                                  |
| 1.026 | Niobium          | Nickel               | 15-20                                  |
| 1.027 | Niobium          | Rhodium              | 15-20                                  |
| 1.028 | Niobium          | Palladium            | 15-20                                  |
| 1.029 | Niobium          | Platinum             | 15-20                                  |
| 1.030 | Niobium          | Copper               | 15-20                                  |
| 1.031 | Niobium          | Silver               | 15-20                                  |
| 1.032 | Niobium          | Gold                 | 15-20                                  |
| 1.033 | Niobium          | Cobalt               | 20-25                                  |
| 1.034 | Niobium          | Nickel               | 20-25                                  |
| 1.035 | Niobium          | Rhodium              | 20-25                                  |
| 1.036 | Niobium          | Palladium            | 20-25                                  |
| 1.037 | Niobium          | Platinum             | 20-25                                  |
| 1.038 | Niobium          | Copper               | 20-25                                  |
| 1.039 | Niobium          | Silver               | 20-25                                  |
| 1.040 | Niobium          | Gold                 | 20-25                                  |
| 1.041 | Niobium          | Cobalt               | 25-30                                  |
| 1.042 | Niobium          | Nickel               | 25-30                                  |
| 1.043 | Niobium          | Rhodium              | 25-30                                  |
| 1.044 | Niobium          | Palladium            | 25-30                                  |
| 1.045 | Niobium          | Platinum             | 25-30                                  |
| 1.046 | Niobium          | Copper               | 25-30                                  |
| 1.047 | Niobium          | Silver               | 25-30                                  |
| 1.048 | Niobium          | Gold                 | 25-30                                  |

Table 2: Table 2 consists of 48 alloys, the refractory metal being tantalum instead of niobium and the non-refractory metal and the amount thereof in wt. % being as indicated in Table 1.

TABLE 2

| No.   | Refractory metal | Non-refractory metal | Amount of non-refractory metal (wt. %) |
|-------|------------------|----------------------|----------------------------------------|
| 2.001 | Tantalum         | Cobalt               | 2-5                                    |
| 2.002 | Tantalum         | Nickel               | 2-5                                    |
| 2.003 | Tantalum         | Rhodium              | 2-5                                    |
| 2.004 | Tantalum         | Palladium            | 2-5                                    |
| 2.005 | Tantalum         | Platinum             | 2-5                                    |
| 2.006 | Tantalum         | Copper               | 2-5                                    |
| 2.007 | Tantalum         | Silver               | 2-5                                    |
| 2.008 | Tantalum         | Gold                 | 2-5                                    |
| 2.009 | Tantalum         | Cobalt               | 5-10                                   |
| 2.010 | Tantalum         | Nickel               | 5-10                                   |
| 2.011 | Tantalum         | Rhodium              | 5-10                                   |

TABLE 2-continued

| No. | Refractory metal | Non-refractory metal | Amount of non-refractory metal (wt. %) |       |
|-----|------------------|----------------------|----------------------------------------|-------|
| 5   | 2.012            | Tantalum             | Palladium                              | 5-10  |
|     | 2.013            | Tantalum             | Platinum                               | 5-10  |
|     | 2.014            | Tantalum             | Copper                                 | 5-10  |
|     | 2.015            | Tantalum             | Silver                                 | 5-10  |
|     | 2.016            | Tantalum             | Gold                                   | 5-10  |
| 10  | 2.017            | Tantalum             | Cobalt                                 | 10-15 |
|     | 2.018            | Tantalum             | Nickel                                 | 10-15 |
|     | 2.019            | Tantalum             | Rhodium                                | 10-15 |
|     | 2.020            | Tantalum             | Palladium                              | 10-15 |
|     | 2.021            | Tantalum             | Platinum                               | 10-15 |
|     | 2.022            | Tantalum             | Copper                                 | 10-15 |
| 15  | 2.023            | Tantalum             | Silver                                 | 10-15 |
|     | 2.024            | Tantalum             | Gold                                   | 10-15 |
|     | 2.025            | Tantalum             | Cobalt                                 | 15-20 |
|     | 2.026            | Tantalum             | Nickel                                 | 15-20 |
|     | 2.027            | Tantalum             | Rhodium                                | 15-20 |
|     | 2.028            | Tantalum             | Palladium                              | 15-20 |
| 20  | 2.029            | Tantalum             | Platinum                               | 15-20 |
|     | 2.030            | Tantalum             | Copper                                 | 15-20 |
|     | 2.031            | Tantalum             | Silver                                 | 15-20 |
|     | 2.032            | Tantalum             | Gold                                   | 15-20 |
|     | 2.033            | Tantalum             | Cobalt                                 | 20-25 |
|     | 2.034            | Tantalum             | Nickel                                 | 20-25 |
|     | 2.035            | Tantalum             | Rhodium                                | 20-25 |
| 25  | 2.036            | Tantalum             | Palladium                              | 20-25 |
|     | 2.037            | Tantalum             | Platinum                               | 20-25 |
|     | 2.038            | Tantalum             | Copper                                 | 20-25 |
|     | 2.039            | Tantalum             | Silver                                 | 20-25 |
|     | 2.040            | Tantalum             | Gold                                   | 20-25 |
|     | 2.041            | Tantalum             | Cobalt                                 | 25-30 |
| 30  | 2.042            | Tantalum             | Nickel                                 | 25-30 |
|     | 2.043            | Tantalum             | Rhodium                                | 25-30 |
|     | 2.044            | Tantalum             | Palladium                              | 25-30 |
|     | 2.045            | Tantalum             | Platinum                               | 25-30 |
|     | 2.046            | Tantalum             | Copper                                 | 25-30 |
|     | 2.047            | Tantalum             | Silver                                 | 25-30 |
| 35  | 2.048            | Tantalum             | Gold                                   | 25-30 |

Table 3: Table 3 consists of 48 alloys, the refractory metal being tungsten instead of niobium and the non-refractory metal and the amount thereof in wt. % being as indicated in Table 1.

TABLE 3

| No. | Refractory metal | Non-refractory metal | Amount of non-refractory metal (wt. %) |       |
|-----|------------------|----------------------|----------------------------------------|-------|
| 45  | 3.001            | Tungsten             | Cobalt                                 | 2-5   |
|     | 3.002            | Tungsten             | Nickel                                 | 2-5   |
|     | 3.003            | Tungsten             | Rhodium                                | 2-5   |
|     | 3.004            | Tungsten             | Palladium                              | 2-5   |
|     | 3.005            | Tungsten             | Platinum                               | 2-5   |
|     | 3.006            | Tungsten             | Copper                                 | 2-5   |
|     | 3.007            | Tungsten             | Silver                                 | 2-5   |
|     | 3.008            | Tungsten             | Gold                                   | 2-5   |
|     | 3.009            | Tungsten             | Cobalt                                 | 5-10  |
|     | 3.010            | Tungsten             | Nickel                                 | 5-10  |
|     | 3.011            | Tungsten             | Rhodium                                | 5-10  |
|     | 3.012            | Tungsten             | Palladium                              | 5-10  |
|     | 3.013            | Tungsten             | Platinum                               | 5-10  |
|     | 3.014            | Tungsten             | Copper                                 | 5-10  |
|     | 3.015            | Tungsten             | Silver                                 | 5-10  |
|     | 3.016            | Tungsten             | Gold                                   | 5-10  |
| 50  | 3.017            | Tungsten             | Cobalt                                 | 10-15 |
|     | 3.018            | Tungsten             | Nickel                                 | 10-15 |
|     | 3.019            | Tungsten             | Rhodium                                | 10-15 |
|     | 3.020            | Tungsten             | Palladium                              | 10-15 |
|     | 3.021            | Tungsten             | Platinum                               | 10-15 |
|     | 3.022            | Tungsten             | Copper                                 | 10-15 |
| 55  | 3.023            | Tungsten             | Silver                                 | 10-15 |
|     | 3.024            | Tungsten             | Gold                                   | 10-15 |

TABLE 3-continued

| No.   | Refractory metal | Non-refractory metal | Amount of non-refractory metal (wt. %) |
|-------|------------------|----------------------|----------------------------------------|
| 3.025 | Tungsten         | Cobalt               | 15-20                                  |
| 3.026 | Tungsten         | Nickel               | 15-20                                  |
| 3.027 | Tungsten         | Rhodium              | 15-20                                  |
| 3.028 | Tungsten         | Palladium            | 15-20                                  |
| 3.029 | Tungsten         | Platinum             | 15-20                                  |
| 3.030 | Tungsten         | Copper               | 15-20                                  |
| 3.031 | Tungsten         | Silver               | 15-20                                  |
| 3.032 | Tungsten         | Gold                 | 15-20                                  |
| 3.033 | Tungsten         | Cobalt               | 20-25                                  |
| 3.034 | Tungsten         | Nickel               | 20-25                                  |
| 3.035 | Tungsten         | Rhodium              | 20-25                                  |
| 3.036 | Tungsten         | Palladium            | 20-25                                  |
| 3.037 | Tungsten         | Platinum             | 20-25                                  |
| 3.038 | Tungsten         | Copper               | 20-25                                  |
| 3.039 | Tungsten         | Silver               | 20-25                                  |
| 3.040 | Tungsten         | Gold                 | 20-25                                  |
| 3.041 | Tungsten         | Cobalt               | 25-30                                  |
| 3.042 | Tungsten         | Nickel               | 25-30                                  |
| 3.043 | Tungsten         | Rhodium              | 25-30                                  |
| 3.044 | Tungsten         | Palladium            | 25-30                                  |
| 3.045 | Tungsten         | Platinum             | 25-30                                  |
| 3.046 | Tungsten         | Copper               | 25-30                                  |
| 3.047 | Tungsten         | Silver               | 25-30                                  |
| 3.048 | Tungsten         | Gold                 | 25-30                                  |

Table 4: Table 4 consists of 48 alloys, the refractory metal being molybdenum instead of niobium and the non-refractory metal and the amount thereof in wt. % being as indicated in Table 1.

TABLE 4

| No.   | Refractory metal | Non-refractory metal | Amount of non-refractory metal (wt. %) |
|-------|------------------|----------------------|----------------------------------------|
| 4,001 | Molybdenum       | Cobalt               | 2-5                                    |
| 4,002 | Molybdenum       | Nickel               | 2-5                                    |
| 4,003 | Molybdenum       | Rhodium              | 2-5                                    |
| 4,004 | Molybdenum       | Palladium            | 2-5                                    |
| 4,005 | Molybdenum       | Platinum             | 2-5                                    |
| 4,006 | Molybdenum       | Copper               | 2-5                                    |
| 4,007 | Molybdenum       | Silver               | 2-5                                    |
| 4,008 | Molybdenum       | Gold                 | 2-5                                    |
| 4,009 | Molybdenum       | Cobalt               | 5-10                                   |
| 4,010 | Molybdenum       | Nickel               | 5-10                                   |
| 4,011 | Molybdenum       | Rhodium              | 5-10                                   |
| 4,012 | Molybdenum       | Palladium            | 5-10                                   |
| 4,013 | Molybdenum       | Platinum             | 5-10                                   |
| 4,014 | Molybdenum       | Copper               | 5-10                                   |
| 4,015 | Molybdenum       | Silver               | 5-10                                   |
| 4,016 | Molybdenum       | Gold                 | 5-10                                   |
| 4,017 | Molybdenum       | Cobalt               | 10-15                                  |
| 4,018 | Molybdenum       | Nickel               | 10-15                                  |
| 4,019 | Molybdenum       | Rhodium              | 10-15                                  |
| 4,020 | Molybdenum       | Palladium            | 10-15                                  |
| 4,021 | Molybdenum       | Platinum             | 10-15                                  |
| 4,022 | Molybdenum       | Copper               | 10-15                                  |
| 4,023 | Molybdenum       | Silver               | 10-15                                  |
| 4,024 | Molybdenum       | Gold                 | 10-15                                  |
| 4,025 | Molybdenum       | Cobalt               | 15-20                                  |
| 4,026 | Molybdenum       | Nickel               | 15-20                                  |
| 4,027 | Molybdenum       | Rhodium              | 15-20                                  |
| 4,028 | Molybdenum       | Palladium            | 15-20                                  |
| 4,029 | Molybdenum       | Platinum             | 15-20                                  |
| 4,030 | Molybdenum       | Copper               | 15-20                                  |
| 4,031 | Molybdenum       | Silver               | 15-20                                  |
| 4,032 | Molybdenum       | Gold                 | 15-20                                  |
| 4,033 | Molybdenum       | Cobalt               | 20-25                                  |
| 4,034 | Molybdenum       | Nickel               | 20-25                                  |
| 4,035 | Molybdenum       | Rhodium              | 20-25                                  |
| 4,036 | Molybdenum       | Palladium            | 20-25                                  |
| 4,037 | Molybdenum       | Platinum             | 20-25                                  |

TABLE 4-continued

| No. | Refractory metal | Non-refractory metal | Amount of non-refractory metal (wt. %) |       |
|-----|------------------|----------------------|----------------------------------------|-------|
| 5   | 4,038            | Molybdenum           | Copper                                 | 20-25 |
|     | 4,039            | Molybdenum           | Silver                                 | 20-25 |
|     | 4,040            | Molybdenum           | Gold                                   | 20-25 |
|     | 4,041            | Molybdenum           | Cobalt                                 | 25-30 |
| 10  | 4,042            | Molybdenum           | Nickel                                 | 25-30 |
|     | 4,043            | Molybdenum           | Rhodium                                | 25-30 |
|     | 4,044            | Molybdenum           | Palladium                              | 25-30 |
|     | 4,045            | Molybdenum           | Platinum                               | 25-30 |
|     | 4,046            | Molybdenum           | Copper                                 | 25-30 |
|     | 4,047            | Molybdenum           | Silver                                 | 25-30 |
| 15  | 4,048            | Molybdenum           | Gold                                   | 25-30 |

Table 5: Table 5 consists of 48 alloys, the refractory metal being titanium instead of niobium and the non-refractory metal and the amount thereof in wt. % being as indicated in Table 1.

TABLE 5

| No. | Refractory metal | Non-refractory metal | Amount of non-refractory metal (wt. %) |       |
|-----|------------------|----------------------|----------------------------------------|-------|
| 25  | 5,001            | Titanium             | Cobalt                                 | 2-5   |
|     | 5,002            | Titanium             | Nickel                                 | 2-5   |
|     | 5,003            | Titanium             | Rhodium                                | 2-5   |
| 30  | 5,004            | Titanium             | Palladium                              | 2-5   |
|     | 5,005            | Titanium             | Platinum                               | 2-5   |
|     | 5,006            | Titanium             | Copper                                 | 2-5   |
|     | 5,007            | Titanium             | Silver                                 | 2-5   |
|     | 5,008            | Titanium             | Gold                                   | 2-5   |
| 35  | 5,009            | Titanium             | Cobalt                                 | 5-10  |
|     | 5,010            | Titanium             | Nickel                                 | 5-10  |
|     | 5,011            | Titanium             | Rhodium                                | 5-10  |
|     | 5,012            | Titanium             | Palladium                              | 5-10  |
| 40  | 5,013            | Titanium             | Platinum                               | 5-10  |
|     | 5,014            | Titanium             | Copper                                 | 5-10  |
|     | 5,015            | Titanium             | Silver                                 | 5-10  |
|     | 5,016            | Titanium             | Gold                                   | 5-10  |
| 45  | 5,017            | Titanium             | Cobalt                                 | 10-15 |
|     | 5,018            | Titanium             | Nickel                                 | 10-15 |
|     | 5,019            | Titanium             | Rhodium                                | 10-15 |
|     | 5,020            | Titanium             | Palladium                              | 10-15 |
|     | 5,021            | Titanium             | Platinum                               | 10-15 |
|     | 5,022            | Titanium             | Copper                                 | 10-15 |
| 50  | 5,023            | Titanium             | Silver                                 | 10-15 |
|     | 5,024            | Titanium             | Gold                                   | 10-15 |
|     | 5,025            | Titanium             | Cobalt                                 | 15-20 |
| 55  | 5,026            | Titanium             | Nickel                                 | 15-20 |
|     | 5,027            | Titanium             | Rhodium                                | 15-20 |
|     | 5,028            | Titanium             | Palladium                              | 15-20 |
| 60  | 5,029            | Titanium             | Platinum                               | 15-20 |
|     | 5,030            | Titanium             | Copper                                 | 15-20 |
|     | 5,031            | Titanium             | Silver                                 | 15-20 |
|     | 5,032            | Titanium             | Gold                                   | 15-20 |
| 65  | 5,033            | Titanium             | Cobalt                                 | 20-25 |
|     | 5,034            | Titanium             | Nickel                                 | 20-25 |
|     | 5,035            | Titanium             | Rhodium                                | 20-25 |
|     | 5,036            | Titanium             | Palladium                              | 20-25 |
|     | 5,037            | Titanium             | Platinum                               | 20-25 |
|     | 5,038            | Titanium             | Copper                                 | 20-25 |
|     | 5,039            | Titanium             | Silver                                 | 20-25 |
|     | 5,040            | Titanium             | Gold                                   | 20-25 |
| 65  | 5,041            | Titanium             | Cobalt                                 | 25-30 |
|     | 5,042            | Titanium             | Nickel                                 | 25-30 |
|     | 5,043            | Titanium             | Rhodium                                | 25-30 |
|     | 5,044            | Titanium             | Palladium                              | 25-30 |
|     | 5,045            | Titanium             | Platinum                               | 25-30 |
|     | 5,046            | Titanium             | Copper                                 | 25-30 |
|     | 5,047            | Titanium             | Silver                                 | 25-30 |
|     | 5,048            | Titanium             | Gold                                   | 25-30 |

Table 6: Table 6 consists of 48 pseudo alloys, the refractory metal being tantalum instead of niobium and the non-refractory metal and the amount thereof in wt. % being as indicated in Table 1.

TABLE 6

| No.   | Refractory metal | Non-refractory metal | Amount of non-   | No.   | Refractory metal | Non-refractory metal | Amount of non- |
|-------|------------------|----------------------|------------------|-------|------------------|----------------------|----------------|
|       |                  |                      | refractory metal |       |                  |                      | (wt. %)        |
| 6.001 | Tantalum         | Cobalt               | 2-5              | 7.008 | Tungsten         | Gold                 | 2-5            |
| 6.002 | Tantalum         | Nickel               | 2-5              | 7.009 | Tungsten         | Cobalt               | 5-10           |
| 6.003 | Tantalum         | Rhodium              | 2-5              | 7.010 | Tungsten         | Nickel               | 5-10           |
| 6.004 | Tantalum         | Palladium            | 2-5              | 7.011 | Tungsten         | Rhodium              | 5-10           |
| 6.005 | Tantalum         | Platinum             | 2-5              | 7.012 | Tungsten         | Palladium            | 5-10           |
| 6.006 | Tantalum         | Copper               | 2-5              | 7.013 | Tungsten         | Platinum             | 5-10           |
| 6.007 | Tantalum         | Silver               | 2-5              | 7.014 | Tungsten         | Copper               | 5-10           |
| 6.008 | Tantalum         | Gold                 | 2-5              | 7.015 | Tungsten         | Silver               | 5-10           |
| 6.009 | Tantalum         | Cobalt               | 5-10             | 7.016 | Tungsten         | Gold                 | 5-10           |
| 6.010 | Tantalum         | Nickel               | 5-10             | 7.017 | Tungsten         | Cobalt               | 10-15          |
| 6.011 | Tantalum         | Rhodium              | 5-10             | 7.018 | Tungsten         | Nickel               | 10-15          |
| 6.012 | Tantalum         | Palladium            | 5-10             | 7.019 | Tungsten         | Rhodium              | 10-15          |
| 6.013 | Tantalum         | Platinum             | 5-10             | 7.020 | Tungsten         | Palladium            | 10-15          |
| 6.014 | Tantalum         | Copper               | 5-10             | 7.021 | Tungsten         | Platinum             | 10-15          |
| 6.015 | Tantalum         | Silver               | 5-10             | 7.022 | Tungsten         | Copper               | 10-15          |
| 6.016 | Tantalum         | Gold                 | 5-10             | 7.023 | Tungsten         | Silver               | 10-15          |
| 6.017 | Tantalum         | Cobalt               | 10-15            | 7.024 | Tungsten         | Gold                 | 10-15          |
| 6.018 | Tantalum         | Nickel               | 10-15            | 7.025 | Tungsten         | Cobalt               | 15-20          |
| 6.019 | Tantalum         | Rhodium              | 10-15            | 7.026 | Tungsten         | Nickel               | 15-20          |
| 6.020 | Tantalum         | Palladium            | 10-15            | 7.027 | Tungsten         | Rhodium              | 15-20          |
| 6.021 | Tantalum         | Platinum             | 10-15            | 7.028 | Tungsten         | Palladium            | 15-20          |
| 6.022 | Tantalum         | Copper               | 10-15            | 7.029 | Tungsten         | Platinum             | 15-20          |
| 6.023 | Tantalum         | Silver               | 10-15            | 7.030 | Tungsten         | Copper               | 15-20          |
| 6.024 | Tantalum         | Gold                 | 10-15            | 7.031 | Tungsten         | Silver               | 15-20          |
| 6.025 | Tantalum         | Cobalt               | 15-20            | 7.032 | Tungsten         | Gold                 | 15-20          |
| 6.026 | Tantalum         | Nickel               | 15-20            | 7.033 | Tungsten         | Cobalt               | 20-25          |
| 6.027 | Tantalum         | Rhodium              | 15-20            | 7.034 | Tungsten         | Nickel               | 20-25          |
| 6.028 | Tantalum         | Palladium            | 15-20            | 7.035 | Tungsten         | Rhodium              | 20-25          |
| 6.029 | Tantalum         | Platinum             | 15-20            | 7.036 | Tungsten         | Palladium            | 20-25          |
| 6.030 | Tantalum         | Copper               | 15-20            | 7.037 | Tungsten         | Platinum             | 20-25          |
| 6.031 | Tantalum         | Silver               | 15-20            | 7.038 | Tungsten         | Copper               | 20-25          |
| 6.032 | Tantalum         | Gold                 | 15-20            | 7.039 | Tungsten         | Silver               | 20-25          |
| 6.033 | Tantalum         | Cobalt               | 20-25            | 7.040 | Tungsten         | Gold                 | 20-25          |
| 6.034 | Tantalum         | Nickel               | 20-25            | 7.041 | Tungsten         | Cobalt               | 25-30          |
| 6.035 | Tantalum         | Rhodium              | 20-25            | 7.042 | Tungsten         | Nickel               | 25-30          |
| 6.036 | Tantalum         | Palladium            | 20-25            | 7.043 | Tungsten         | Rhodium              | 25-30          |
| 6.037 | Tantalum         | Platinum             | 20-25            | 7.044 | Tungsten         | Palladium            | 25-30          |
| 6.038 | Tantalum         | Copper               | 20-25            | 7.045 | Tungsten         | Platinum             | 25-30          |
| 6.039 | Tantalum         | Silver               | 20-25            | 7.046 | Tungsten         | Copper               | 25-30          |
| 6.040 | Tantalum         | Gold                 | 20-25            | 7.047 | Tungsten         | Silver               | 25-30          |
| 6.041 | Tantalum         | Cobalt               | 25-30            | 7.048 | Tungsten         | Gold                 | 25-30          |
| 6.042 | Tantalum         | Nickel               | 25-30            |       |                  |                      |                |
| 6.043 | Tantalum         | Rhodium              | 25-30            |       |                  |                      |                |
| 6.044 | Tantalum         | Palladium            | 25-30            |       |                  |                      |                |
| 6.045 | Tantalum         | Platinum             | 25-30            |       |                  |                      |                |
| 6.046 | Tantalum         | Copper               | 25-30            |       |                  |                      |                |
| 6.047 | Tantalum         | Silver               | 25-30            |       |                  |                      |                |
| 6.048 | Tantalum         | Gold                 | 25-30            |       |                  |                      |                |

Table 7: Table 7 consists of 48 pseudo alloys, the refractory metal being tungsten instead of niobium and the non-refractory metal and the amount thereof in wt. % being as indicated in Table 1.

TABLE 7

| No.   | Refractory metal | Non-refractory metal | Amount of non-   | No.   | Refractory metal | Non-refractory metal | Amount of non- |
|-------|------------------|----------------------|------------------|-------|------------------|----------------------|----------------|
|       |                  |                      | refractory metal |       |                  |                      | (wt. %)        |
| 7.001 | Tungsten         | Cobalt               | 2-5              | 8.001 | Molybdenum       | Cobalt               | 2-5            |
| 7.002 | Tungsten         | Nickel               | 2-5              | 8.002 | Molybdenum       | Nickel               | 2-5            |
| 7.003 | Tungsten         | Rhodium              | 2-5              | 8.003 | Molybdenum       | Rhodium              | 2-5            |
| 7.004 | Tungsten         | Palladium            | 2-5              | 8.004 | Molybdenum       | Palladium            | 2-5            |
| 7.005 | Tungsten         | Platinum             | 2-5              | 8.005 | Molybdenum       | Platinum             | 2-5            |
| 7.006 | Tungsten         | Copper               | 2-5              | 8.006 | Molybdenum       | Copper               | 2-5            |
| 7.007 | Tungsten         | Silver               | 2-5              | 8.007 | Molybdenum       | Silver               | 2-5            |

TABLE 7-continued

| 5  | No.   | Refractory metal | Non-refractory metal | Amount of non-   |
|----|-------|------------------|----------------------|------------------|
|    |       |                  |                      | refractory metal |
| 5  | 7.008 | Tungsten         | Gold                 | 2-5              |
| 5  | 7.009 | Tungsten         | Cobalt               | 5-10             |
| 5  | 7.010 | Tungsten         | Nickel               | 5-10             |
| 5  | 7.011 | Tungsten         | Rhodium              | 5-10             |
| 5  | 7.012 | Tungsten         | Palladium            | 5-10             |
| 5  | 7.013 | Tungsten         | Platinum             | 5-10             |
| 10 | 7.014 | Tungsten         | Copper               | 5-10             |
| 10 | 7.015 | Tungsten         | Silver               | 5-10             |
| 10 | 7.016 | Tungsten         | Gold                 | 5-10             |
| 10 | 7.017 | Tungsten         | Cobalt               | 10-15            |
| 10 | 7.018 | Tungsten         | Nickel               | 10-15            |
| 10 | 7.019 | Tungsten         | Rhodium              | 10-15            |
| 10 | 7.020 | Tungsten         | Palladium            | 10-15            |
| 10 | 7.021 | Tungsten         | Platinum             | 10-15            |
| 10 | 7.022 | Tungsten         | Copper               | 10-15            |
| 10 | 7.023 | Tungsten         | Silver               | 10-15            |
| 10 | 7.024 | Tungsten         | Gold                 | 10-15            |
| 10 | 7.025 | Tungsten         | Cobalt               | 15-20            |
| 15 | 7.026 | Tungsten         | Nickel               | 15-20            |
| 15 | 7.027 | Tungsten         | Rhodium              | 15-20            |
| 15 | 7.028 | Tungsten         | Palladium            | 15-20            |
| 15 | 7.029 | Tungsten         | Platinum             | 15-20            |
| 15 | 7.030 | Tungsten         | Copper               | 15-20            |
| 15 | 7.031 | Tungsten         | Silver               | 15-20            |
| 15 | 7.032 | Tungsten         | Gold                 | 15-20            |
| 20 | 7.033 | Tungsten         | Cobalt               | 20-25            |
| 20 | 7.034 | Tungsten         | Nickel               | 20-25            |
| 20 | 7.035 | Tungsten         | Rhodium              | 20-25            |
| 20 | 7.036 | Tungsten         | Palladium            | 20-25            |
| 20 | 7.037 | Tungsten         | Platinum             | 20-25            |
| 20 | 7.038 | Tungsten         | Copper               | 20-25            |
| 20 | 7.039 | Tungsten         | Silver               | 20-25            |
| 20 | 7.040 | Tungsten         | Gold                 | 20-25            |
| 20 | 7.041 | Tungsten         | Cobalt               | 25-30            |
| 25 | 7.042 | Tungsten         | Nickel               | 25-30            |
| 25 | 7.043 | Tungsten         | Rhodium              | 25-30            |
| 25 | 7.044 | Tungsten         | Palladium            | 25-30            |
| 25 | 7.045 | Tungsten         | Platinum             | 25-30            |
| 25 | 7.046 | Tungsten         | Copper               | 25-30            |
| 25 | 7.047 | Tungsten         | Silver               | 25-30            |
| 25 | 7.048 | Tungsten         | Gold                 | 25-30            |

40 Table 8: Table 8 consists of 48 pseudo alloys, the refractory metal being molybdenum instead of niobium and the non-refractory metal and the amount thereof in wt. % being as indicated in Table 1.

| 45 | No.   | Refractory metal | Non-refractory metal | Amount of non-   |
|----|-------|------------------|----------------------|------------------|
|    |       |                  |                      | refractory metal |
| 50 | 8.001 | Molybdenum       | Cobalt               | 2-5              |
| 50 | 8.002 | Molybdenum       | Nickel               | 2-5              |
| 50 | 8.003 | Molybdenum       | Rhodium              | 2-5              |
| 50 | 8.004 | Molybdenum       | Palladium            | 2-5              |
| 50 | 8.005 | Molybdenum       | Platinum             | 2-5              |
| 50 | 8.006 | Molybdenum       | Copper               | 2-5              |
| 50 | 8.007 | Molybdenum       | Silver               | 2-5              |
| 50 | 8.008 | Molybdenum       | Gold                 | 2-5              |
| 50 | 8.009 | Molybdenum       | Cobalt               | 5-10             |
| 50 | 8.010 | Molybdenum       | Nickel               | 5-10             |
| 50 | 8.011 | Molybdenum       | Rhodium              | 5-10             |
| 50 | 8.012 | Molybdenum       | Palladium            | 5-10             |
| 50 | 8.013 | Molybdenum       | Platinum             | 5-10             |
| 50 | 8.014 | Molybdenum       | Copper               | 5-10             |
| 50 | 8.015 | Molybdenum       | Silver               | 5-10             |
| 50 | 8.016 | Molybdenum       | Gold                 | 5-10             |
| 50 | 8.017 | Molybdenum       | Cobalt               | 10-15            |
| 50 | 8.018 | Molybdenum       | Nickel               | 10-15            |
| 50 | 8.019 | Molybdenum       | Rhodium              | 10-15            |
| 50 | 8.020 | Molybdenum       | Palladium            | 10-15            |

TABLE 7

| No.   | Refractory metal | Non-refractory metal | Amount of non-   |
|-------|------------------|----------------------|------------------|
|       |                  |                      | refractory metal |
| 7.001 | Tungsten         | Cobalt               | 2-5              |
| 7.002 | Tungsten         | Nickel               | 2-5              |
| 7.003 | Tungsten         | Rhodium              | 2-5              |
| 7.004 | Tungsten         | Palladium            | 2-5              |
| 7.005 | Tungsten         | Platinum             | 2-5              |
| 7.006 | Tungsten         | Copper               | 2-5              |
| 7.007 | Tungsten         | Silver               | 2-5              |

TABLE 8-continued

| No.   | Refractory metal | Non-refractory metal | Amount of non-refractory metal (wt. %) |
|-------|------------------|----------------------|----------------------------------------|
| 8.021 | Molybdenum       | Platinum             | 10-15                                  |
| 8.022 | Molybdenum       | Copper               | 10-15                                  |
| 8.023 | Molybdenum       | Silver               | 10-15                                  |
| 8.024 | Molybdenum       | Gold                 | 10-15                                  |
| 8.025 | Molybdenum       | Cobalt               | 15-20                                  |
| 8.026 | Molybdenum       | Nickel               | 15-20                                  |
| 8.027 | Molybdenum       | Rhodium              | 15-20                                  |
| 8.028 | Molybdenum       | Palladium            | 15-20                                  |
| 8.029 | Molybdenum       | Platinum             | 15-20                                  |
| 8.030 | Molybdenum       | Copper               | 15-20                                  |
| 8.031 | Molybdenum       | Silver               | 15-20                                  |
| 8.032 | Molybdenum       | Gold                 | 15-20                                  |
| 8.033 | Molybdenum       | Cobalt               | 20-25                                  |
| 8.034 | Molybdenum       | Nickel               | 20-25                                  |
| 8.035 | Molybdenum       | Rhodium              | 20-25                                  |
| 8.036 | Molybdenum       | Palladium            | 20-25                                  |
| 8.037 | Molybdenum       | Platinum             | 20-25                                  |
| 8.038 | Molybdenum       | Copper               | 20-25                                  |
| 8.039 | Molybdenum       | Silver               | 20-25                                  |
| 8.040 | Molybdenum       | Gold                 | 20-25                                  |
| 8.041 | Molybdenum       | Cobalt               | 25-30                                  |
| 8.042 | Molybdenum       | Nickel               | 25-30                                  |
| 8.043 | Molybdenum       | Rhodium              | 25-30                                  |
| 8.044 | Molybdenum       | Palladium            | 25-30                                  |
| 8.045 | Molybdenum       | Platinum             | 25-30                                  |
| 8.046 | Molybdenum       | Copper               | 25-30                                  |
| 8.047 | Molybdenum       | Silver               | 25-30                                  |
| 8.048 | Molybdenum       | Gold                 | 25-30                                  |

Table 9: Table 9 consists of 48 pseudo alloys, the refractory metal being titanium instead of niobium and the non-refractory metal and the amount thereof in wt. % being as indicated in Table 1.

TABLE 9

| No.   | Refractory metal | Non-refractory metal | Amount of non-refractory metal (wt.%) |
|-------|------------------|----------------------|---------------------------------------|
| 9.001 | Titanium         | Cobalt               | 2-5                                   |
| 9.002 | Titanium         | Nickel               | 2-5                                   |
| 9.003 | Titanium         | Rhodium              | 2-5                                   |
| 9.004 | Titanium         | Palladium            | 2-5                                   |
| 9.005 | Titanium         | Platinum             | 2-5                                   |
| 9.006 | Titanium         | Copper               | 2-5                                   |
| 9.007 | Titanium         | Silver               | 2-5                                   |
| 9.008 | Titanium         | Gold                 | 2-5                                   |
| 9.009 | Titanium         | Cobalt               | 5-10                                  |
| 9.010 | Titanium         | Nickel               | 5-10                                  |
| 9.011 | Titanium         | Rhodium              | 5-10                                  |
| 9.012 | Titanium         | Palladium            | 5-10                                  |
| 9.013 | Titanium         | Platinum             | 5-10                                  |
| 9.014 | Titanium         | Copper               | 5-10                                  |
| 9.015 | Titanium         | Silver               | 5-10                                  |
| 9.016 | Titanium         | Gold                 | 5-10                                  |
| 9.017 | Titanium         | Cobalt               | 10-15                                 |
| 9.018 | Titanium         | Nickel               | 10-15                                 |
| 9.019 | Titanium         | Rhodium              | 10-15                                 |
| 9.020 | Titanium         | Palladium            | 10-15                                 |
| 9.021 | Titanium         | Platinum             | 10-15                                 |
| 9.022 | Titanium         | Copper               | 10-15                                 |
| 9.023 | Titanium         | Silver               | 10-15                                 |
| 9.024 | Titanium         | Gold                 | 10-15                                 |
| 9.025 | Titanium         | Cobalt               | 15-20                                 |
| 9.026 | Titanium         | Nickel               | 15-20                                 |
| 9.027 | Titanium         | Rhodium              | 15-20                                 |
| 9.028 | Titanium         | Palladium            | 15-20                                 |
| 9.029 | Titanium         | Platinum             | 15-20                                 |
| 9.030 | Titanium         | Copper               | 15-20                                 |
| 9.031 | Titanium         | Silver               | 15-20                                 |
| 9.032 | Titanium         | Gold                 | 15-20                                 |
| 9.033 | Titanium         | Cobalt               | 20-25                                 |

TABLE 9-continued

| No.   | Refractory metal | Non-refractory metal | Amount of non-refractory metal (wt.%) |
|-------|------------------|----------------------|---------------------------------------|
| 5     | 9.034            | Titanium             | Nickel                                |
| 9.035 | Titanium         | Rhodium              | 20-25                                 |
| 9.036 | Titanium         | Palladium            | 20-25                                 |
| 9.037 | Titanium         | Platinum             | 20-25                                 |
| 9.038 | Titanium         | Copper               | 20-25                                 |
| 9.039 | Titanium         | Silver               | 20-25                                 |
| 9.040 | Titanium         | Gold                 | 20-25                                 |
| 9.041 | Titanium         | Cobalt               | 25-30                                 |
| 9.042 | Titanium         | Nickel               | 25-30                                 |
| 9.043 | Titanium         | Rhodium              | 25-30                                 |
| 9.044 | Titanium         | Palladium            | 25-30                                 |
| 9.045 | Titanium         | Platinum             | 25-30                                 |
| 9.046 | Titanium         | Copper               | 25-30                                 |
| 9.047 | Titanium         | Silver               | 25-30                                 |
| 9.048 | Titanium         | Gold                 | 25-30                                 |

20 Table 10: Table 10 consists of 48 powder mixtures, the refractory metal being tantalum instead of niobium and the non-refractory metal and the amount thereof in wt. % being as indicated in Table 1.

TABLE 10

| No.    | Refractory metal | Non-refractory metal | Amount of non-refractory metal (wt.%) |
|--------|------------------|----------------------|---------------------------------------|
| 30     | 10.001           | Tantalum             | Cobalt                                |
| 10.002 | Tantalum         | Nickel               | 2-5                                   |
| 10.003 | Tantalum         | Rhodium              | 2-5                                   |
| 10.004 | Tantalum         | Palladium            | 2-5                                   |
| 10.005 | Tantalum         | Platinum             | 2-5                                   |
| 10.006 | Tantalum         | Copper               | 2-5                                   |
| 10.007 | Tantalum         | Silver               | 2-5                                   |
| 10.008 | Tantalum         | Gold                 | 2-5                                   |
| 10.009 | Tantalum         | Cobalt               | 5-10                                  |
| 10.010 | Tantalum         | Nickel               | 5-10                                  |
| 10.011 | Tantalum         | Rhodium              | 5-10                                  |
| 10.012 | Tantalum         | Palladium            | 5-10                                  |
| 10.013 | Tantalum         | Platinum             | 5-10                                  |
| 35     | 10.014           | Tantalum             | Copper                                |
| 10.015 | Tantalum         | Silver               | 5-10                                  |
| 10.016 | Tantalum         | Gold                 | 5-10                                  |
| 10.017 | Tantalum         | Cobalt               | 10-15                                 |
| 10.018 | Tantalum         | Nickel               | 10-15                                 |
| 10.019 | Tantalum         | Rhodium              | 10-15                                 |
| 40     | 10.020           | Tantalum             | Palladium                             |
| 10.021 | Tantalum         | Platinum             | 10-15                                 |
| 10.022 | Tantalum         | Copper               | 10-15                                 |
| 10.023 | Tantalum         | Silver               | 10-15                                 |
| 10.024 | Tantalum         | Gold                 | 10-15                                 |
| 10.025 | Tantalum         | Cobalt               | 15-20                                 |
| 45     | 10.026           | Tantalum             | Nickel                                |
| 10.027 | Tantalum         | Rhodium              | 15-20                                 |
| 10.028 | Tantalum         | Palladium            | 15-20                                 |
| 10.029 | Tantalum         | Platinum             | 15-20                                 |
| 10.030 | Tantalum         | Copper               | 15-20                                 |
| 10.031 | Tantalum         | Silver               | 15-20                                 |
| 10.032 | Tantalum         | Gold                 | 15-20                                 |
| 50     | 10.033           | Tantalum             | Cobalt                                |
| 10.034 | Tantalum         | Nickel               | 20-25                                 |
| 10.035 | Tantalum         | Rhodium              | 20-25                                 |
| 10.036 | Tantalum         | Palladium            | 20-25                                 |
| 10.037 | Tantalum         | Platinum             | 20-25                                 |
| 10.038 | Tantalum         | Copper               | 20-25                                 |
| 55     | 10.039           | Tantalum             | Silver                                |
| 10.040 | Tantalum         | Gold                 | 20-25                                 |
| 10.041 | Tantalum         | Cobalt               | 25-30                                 |
| 10.042 | Tantalum         | Nickel               | 25-30                                 |
| 10.043 | Tantalum         | Rhodium              | 25-30                                 |
| 60     | 10.044           | Tantalum             | Palladium                             |
| 10.045 | Tantalum         | Platinum             | 25-30                                 |
| 10.046 | Tantalum         | Copper               | 25-30                                 |
| 65     | 10.047           | Tantalum             |                                       |

TABLE 10-continued

| No.    | Refractory metal | Non-refractory metal | Amount of non-refractory metal (wt.%) |
|--------|------------------|----------------------|---------------------------------------|
|        |                  |                      |                                       |
| 10.047 | Tantalum         | Silver               | 25-30                                 |
| 10.048 | Tantalum         | Gold                 | 25-30                                 |

Table 11: Table 11 consists of 48 powder mixtures, the refractory metal being tungsten instead of niobium and the non-refractory metal and the amount thereof in wt. % being as indicated in Table 1.

TABLE 11

| No.    | Refractory metal | Non-refractory metal | Amount of non-refractory metal (wt.%) |
|--------|------------------|----------------------|---------------------------------------|
|        |                  |                      |                                       |
| 11.001 | Tungsten         | Cobalt               | 2-5                                   |
| 11.002 | Tungsten         | Nickel               | 2-5                                   |
| 11.003 | Tungsten         | Rhodium              | 2-5                                   |
| 11.004 | Tungsten         | Palladium            | 2-5                                   |
| 11.005 | Tungsten         | Platinum             | 2-5                                   |
| 11.006 | Tungsten         | Copper               | 2-5                                   |
| 11.007 | Tungsten         | Silver               | 2-5                                   |
| 11.008 | Tungsten         | Gold                 | 2-5                                   |
| 11.009 | Tungsten         | Cobalt               | 5-10                                  |
| 11.010 | Tungsten         | Nickel               | 5-10                                  |
| 11.011 | Tungsten         | Rhodium              | 5-10                                  |
| 11.012 | Tungsten         | Palladium            | 5-10                                  |
| 11.013 | Tungsten         | Platinum             | 5-10                                  |
| 11.014 | Tungsten         | Copper               | 5-10                                  |
| 11.015 | Tungsten         | Silver               | 5-10                                  |
| 11.016 | Tungsten         | Gold                 | 5-10                                  |
| 11.017 | Tungsten         | Cobalt               | 10-15                                 |
| 11.018 | Tungsten         | Nickel               | 10-15                                 |
| 11.019 | Tungsten         | Rhodium              | 10-15                                 |
| 11.020 | Tungsten         | Palladium            | 10-15                                 |
| 11.021 | Tungsten         | Platinum             | 10-15                                 |
| 11.022 | Tungsten         | Copper               | 10-15                                 |
| 11.023 | Tungsten         | Silver               | 10-15                                 |
| 11.024 | Tungsten         | Gold                 | 10-15                                 |
| 11.025 | Tungsten         | Cobalt               | 15-20                                 |
| 11.026 | Tungsten         | Nickel               | 15-20                                 |
| 11.027 | Tungsten         | Rhodium              | 15-20                                 |
| 11.028 | Tungsten         | Palladium            | 15-20                                 |
| 11.029 | Tungsten         | Platinum             | 15-20                                 |
| 11.030 | Tungsten         | Copper               | 15-20                                 |
| 11.031 | Tungsten         | Silver               | 15-20                                 |
| 11.032 | Tungsten         | Gold                 | 15-20                                 |
| 11.033 | Tungsten         | Cobalt               | 20-25                                 |
| 11.034 | Tungsten         | Nickel               | 20-25                                 |
| 11.035 | Tungsten         | Rhodium              | 20-25                                 |
| 11.036 | Tungsten         | Palladium            | 20-25                                 |
| 11.037 | Tungsten         | Platinum             | 20-25                                 |
| 11.038 | Tungsten         | Copper               | 20-25                                 |
| 11.039 | Tungsten         | Silver               | 20-25                                 |
| 11.040 | Tungsten         | Gold                 | 20-25                                 |
| 11.041 | Tungsten         | Cobalt               | 25-30                                 |
| 11.042 | Tungsten         | Nickel               | 25-30                                 |
| 11.043 | Tungsten         | Rhodium              | 25-30                                 |
| 11.044 | Tungsten         | Palladium            | 25-30                                 |
| 11.045 | Tungsten         | Platinum             | 25-30                                 |
| 11.046 | Tungsten         | Copper               | 25-30                                 |
| 11.047 | Tungsten         | Silver               | 25-30                                 |
| 11.048 | Tungsten         | Gold                 | 25-30                                 |

Table 12: Table 12 consists of 48 powder mixtures, the refractory metal being molybdenum instead of niobium and the non-refractory metal and the amount thereof in wt. % being as indicated in Table 1.

TABLE 12

| No.    | Refractory metal | Non-refractory metal | Amount of non-refractory metal (wt.%) |
|--------|------------------|----------------------|---------------------------------------|
| 5      |                  |                      |                                       |
| 12.001 | Molybdenum       | Cobalt               | 2-5                                   |
| 12.002 | Molybdenum       | Nickel               | 2-5                                   |
| 12.003 | Molybdenum       | Rhodium              | 2-5                                   |
| 12.004 | Molybdenum       | Palladium            | 2-5                                   |
| 12.005 | Molybdenum       | Platinum             | 2-5                                   |
| 12.006 | Molybdenum       | Copper               | 2-5                                   |
| 12.007 | Molybdenum       | Silver               | 2-5                                   |
| 12.008 | Molybdenum       | Gold                 | 2-5                                   |
| 12.009 | Molybdenum       | Cobalt               | 5-10                                  |
| 12.010 | Molybdenum       | Nickel               | 5-10                                  |
| 12.011 | Molybdenum       | Rhodium              | 5-10                                  |
| 12.012 | Molybdenum       | Palladium            | 5-10                                  |
| 12.013 | Molybdenum       | Platinum             | 5-10                                  |
| 12.014 | Molybdenum       | Copper               | 5-10                                  |
| 12.015 | Molybdenum       | Silver               | 5-10                                  |
| 12.016 | Molybdenum       | Gold                 | 5-10                                  |
| 12.017 | Molybdenum       | Cobalt               | 10-15                                 |
| 12.018 | Molybdenum       | Nickel               | 10-15                                 |
| 12.019 | Molybdenum       | Rhodium              | 10-15                                 |
| 12.020 | Molybdenum       | Palladium            | 10-15                                 |
| 12.021 | Molybdenum       | Platinum             | 10-15                                 |
| 12.022 | Molybdenum       | Copper               | 10-15                                 |
| 12.023 | Molybdenum       | Silver               | 10-15                                 |
| 12.024 | Molybdenum       | Gold                 | 10-15                                 |
| 12.025 | Molybdenum       | Cobalt               | 15-20                                 |
| 12.026 | Molybdenum       | Nickel               | 15-20                                 |
| 12.027 | Molybdenum       | Rhodium              | 15-20                                 |
| 12.028 | Molybdenum       | Palladium            | 15-20                                 |
| 12.029 | Molybdenum       | Platinum             | 15-20                                 |
| 12.030 | Molybdenum       | Copper               | 15-20                                 |
| 12.031 | Molybdenum       | Silver               | 15-20                                 |
| 12.032 | Molybdenum       | Gold                 | 15-20                                 |
| 12.033 | Molybdenum       | Cobalt               | 20-25                                 |
| 12.034 | Molybdenum       | Nickel               | 20-25                                 |
| 12.035 | Molybdenum       | Rhodium              | 20-25                                 |
| 12.036 | Molybdenum       | Palladium            | 20-25                                 |
| 12.037 | Molybdenum       | Platinum             | 20-25                                 |
| 12.038 | Molybdenum       | Copper               | 20-25                                 |
| 12.039 | Molybdenum       | Silver               | 20-25                                 |
| 12.040 | Molybdenum       | Gold                 | 20-25                                 |
| 12.041 | Molybdenum       | Cobalt               | 25-30                                 |
| 12.042 | Molybdenum       | Nickel               | 25-30                                 |
| 12.043 | Molybdenum       | Rhodium              | 25-30                                 |
| 12.044 | Molybdenum       | Palladium            | 25-30                                 |
| 12.045 | Molybdenum       | Platinum             | 25-30                                 |
| 12.046 | Molybdenum       | Copper               | 25-30                                 |
| 12.047 | Molybdenum       | Silver               | 25-30                                 |
| 12.048 | Molybdenum       | Gold                 | 25-30                                 |
| 45     |                  |                      |                                       |
| 13.001 | Titanium         | Cobalt               | 2-5                                   |
| 13.002 | Titanium         | Nickel               | 2-5                                   |
| 13.003 | Titanium         | Rhodium              | 2-5                                   |
| 13.004 | Titanium         | Palladium            | 2-5                                   |
| 13.005 | Titanium         | Platinum             | 2-5                                   |
| 13.006 | Titanium         | Copper               | 2-5                                   |
| 13.007 | Titanium         | Silver               | 2-5                                   |
| 13.008 | Titanium         | Gold                 | 2-5                                   |
| 13.009 | Titanium         | Cobalt               | 5-10                                  |
| 13.010 | Titanium         | Nickel               | 5-10                                  |
| 13.011 | Titanium         | Rhodium              | 5-10                                  |
| 13.012 | Titanium         | Palladium            | 5-10                                  |
| 13.013 | Titanium         | Platinum             | 5-10                                  |
| 50     |                  |                      |                                       |
| 11.027 | Tungsten         | Rhodium              | 15-20                                 |
| 11.028 | Tungsten         | Palladium            | 15-20                                 |
| 11.029 | Tungsten         | Platinum             | 15-20                                 |
| 11.030 | Tungsten         | Copper               | 15-20                                 |
| 11.031 | Tungsten         | Silver               | 15-20                                 |
| 11.032 | Tungsten         | Gold                 | 15-20                                 |
| 11.033 | Tungsten         | Cobalt               | 20-25                                 |
| 11.034 | Tungsten         | Nickel               | 20-25                                 |
| 11.035 | Tungsten         | Rhodium              | 20-25                                 |
| 11.036 | Tungsten         | Palladium            | 20-25                                 |
| 11.037 | Tungsten         | Platinum             | 20-25                                 |
| 11.038 | Tungsten         | Copper               | 20-25                                 |
| 11.039 | Tungsten         | Silver               | 20-25                                 |
| 11.040 | Tungsten         | Gold                 | 20-25                                 |
| 11.041 | Tungsten         | Cobalt               | 25-30                                 |
| 11.042 | Tungsten         | Nickel               | 25-30                                 |
| 11.043 | Tungsten         | Rhodium              | 25-30                                 |
| 11.044 | Tungsten         | Palladium            | 25-30                                 |
| 11.045 | Tungsten         | Platinum             | 25-30                                 |
| 11.046 | Tungsten         | Copper               | 25-30                                 |
| 11.047 | Tungsten         | Silver               | 25-30                                 |
| 11.048 | Tungsten         | Gold                 | 25-30                                 |
| 55     |                  |                      |                                       |
| 13.001 | Titanium         | Cobalt               | 2-5                                   |
| 13.002 | Titanium         | Nickel               | 2-5                                   |
| 13.003 | Titanium         | Rhodium              | 2-5                                   |
| 13.004 | Titanium         | Palladium            | 2-5                                   |
| 13.005 | Titanium         | Platinum             | 2-5                                   |
| 13.006 | Titanium         | Copper               | 2-5                                   |
| 13.007 | Titanium         | Silver               | 2-5                                   |
| 13.008 | Titanium         | Gold                 | 2-5                                   |
| 13.009 | Titanium         | Cobalt               | 5-10                                  |
| 13.010 | Titanium         | Nickel               | 5-10                                  |
| 13.011 | Titanium         | Rhodium              | 5-10                                  |
| 13.012 | Titanium         | Palladium            | 5-10                                  |
| 13.013 | Titanium         | Platinum             | 5-10                                  |
| 60     |                  |                      |                                       |
| 11.049 | Tungsten         | Rhodium              | 15-20                                 |
| 11.050 | Tungsten         | Palladium            | 15-20                                 |
| 11.051 | Tungsten         | Platinum             | 15-20                                 |
| 11.052 | Tungsten         | Copper               | 15-20                                 |
| 11.053 | Tungsten         | Silver               | 15-20                                 |
| 11.054 | Tungsten         | Gold                 | 15-20                                 |
| 11.055 | Tungsten         | Cobalt               | 20-25                                 |
| 11.056 | Tungsten         | Nickel               | 20-25                                 |
| 11.057 | Tungsten         | Rhodium              | 20-25                                 |
| 11.058 | Tungsten         | Palladium            | 20-25                                 |
| 11.059 | Tungsten         | Platinum             | 20-25                                 |
| 11.060 | Tungsten         | Copper               | 20-25                                 |
| 11.061 | Tungsten         | Silver               | 20-25                                 |
| 11.062 | Tungsten         | Gold                 | 20-25                                 |
| 11.063 | Tungsten         | Cobalt               | 25-30                                 |
| 11.064 | Tungsten         | Nickel               | 25-30                                 |
| 11.065 | Tungsten         | Rhodium              | 25-30                                 |
| 11.066 | Tungsten         | Palladium            | 25-30                                 |
| 11.067 | Tungsten         | Platinum             | 25-30                                 |
| 11.068 | Tungsten         | Copper               | 25-30                                 |
| 11.069 | Tungsten         | Silver               | 25-30                                 |
| 11.070 | Tungsten         | Gold                 | 25-30                                 |
| 11.071 | Tungsten         | Cobalt               | 30-35                                 |
| 11.072 | Tungsten         | Nickel               | 30-35                                 |
| 11.073 | Tungsten         | Rhodium              | 30-35                                 |
| 11.074 | Tungsten         | Palladium            | 30-35                                 |
| 11.075 | Tungsten         | Platinum             | 30-35                                 |
| 11.076 | Tungsten         | Copper               | 30-35                                 |
| 11.077 | Tungsten         | Silver               | 30-35                                 |
| 11.078 | Tungsten         | Gold                 | 30-35                                 |
| 11.079 | Tungsten         | Cobalt               | 35-40                                 |
| 11.080 | Tungsten         | Nickel               | 35-40                                 |
| 11.081 | Tungsten         | Rhodium              | 35-40                                 |
| 11.082 | Tungsten         | Palladium            | 35-40                                 |
| 11.083 | Tungsten         | Platinum             | 35-40                                 |
| 11.084 | Tungsten         | Copper               | 35-40                                 |
| 11.085 | Tungsten         | Silver               | 35-40                                 |
| 11.086 | Tungsten         | Gold                 | 35-40                                 |
| 11.087 | Tungsten         | Cobalt               | 40-45                                 |
| 11.088 | Tungsten         | Nickel               | 40-45                                 |
| 11.089 | Tungsten         | Rhodium              | 40-45                                 |
| 11.090 | Tungsten         | Palladium            | 40-45                                 |
| 11.091 | Tungsten         | Platinum             | 40-45                                 |
| 11.092 | Tungsten         | Copper               | 40-45                                 |
| 11.093 | Tungsten         | Silver               | 40-45                                 |
| 11.094 | Tungsten         | Gold                 | 40-45                                 |
| 11.095 | Tungsten         | Cobalt               | 45-50                                 |
| 11.096 | Tungsten         | Nickel               | 45-50                                 |
| 11.097 | Tungsten         | Rhodium              | 45-50                                 |
| 11.098 | Tungsten         | Palladium            | 45-50                                 |
| 11.099 | Tungsten         | Platinum             | 45-50                                 |
| 11.100 | Tungsten         | Copper               | 45-50                                 |
| 11.101 | Tungsten         | Silver               | 45-50                                 |
| 11.102 | Tungsten         | Gold                 | 45-50                                 |
| 11.103 | Tungsten         | Cobalt               | 50-55                                 |
| 11.104 | Tungsten         | Nickel               | 50-55                                 |
| 11.105 | Tungsten         | Rhodium              | 50-55                                 |
| 11.106 | Tungsten         | Palladium            | 50-55                                 |
| 11.107 | Tungsten         | Platinum             | 50-55                                 |
| 11.108 | Tungsten         | Copper               | 50-55                                 |
| 11.109 | Tungsten         | Silver               | 50-55                                 |
| 11.110 | Tungsten         | Gold                 | 50-55                                 |
| 11.111 | Tungsten         | Cobalt               | 55-60                                 |
| 11.112 | Tungsten         | Nickel               | 55-60                                 |
| 11.113 | Tungsten         | Rhodium              | 55-60                                 |
| 11.114 | Tungsten         | Palladium            | 55-60                                 |
| 11.115 | Tungsten         | Platinum             | 55-60                                 |
| 11.116 | Tungsten         | Copper               | 55-60                                 |
| 11.117 | Tungsten         | Silver               | 55-60                                 |
| 11.118 | Tungsten         | Gold                 | 55-60                                 |
| 11.119 | Tungsten         | Cobalt               | 60-65                                 |
| 11.120 | Tungsten         | Nickel               | 60-65                                 |
| 11.121 | Tungsten         | Rhodium              | 60-65                                 |
| 11.122 | Tungsten         | Palladium            | 60-65                                 |
| 11.123 | Tungsten         | Platinum             | 60-65                                 |
| 11.124 | Tungsten         | Copper               | 60-65                                 |
| 11.125 | Tungsten         | Silver               | 60-65                                 |
| 11.126 | Tungsten         | Gold                 | 60-65                                 |
| 11.127 | Tungsten         | Cobalt               | 65-70                                 |
| 11.128 | Tungsten         | Nickel               | 65-70                                 |
| 11.129 | Tungsten         | Rhodium              | 65-70                                 |
| 11.130 | Tungsten         | Palladium            | 65-70                                 |
| 11.131 | Tungsten         | Platinum             | 65-70                                 |
| 11.132 | Tungsten         | Copper               | 65-70                                 |
| 11.133 | Tungsten         | Silver               | 65-70                                 |
| 11.134 | Tungsten         | Gold                 | 65-70                                 |
| 11.135 | Tungsten         | Cobalt               | 70-75                                 |
| 11.136 | Tungsten         | Nickel               | 70-75                                 |
| 11.137 | Tungsten         | Rhodium              | 70-75                                 |
| 11.138 | Tungsten         | Palladium            | 70-75                                 |
| 11.139 | Tungsten         | Platinum             | 70-75                                 |
| 11.140 | Tungsten         | Copper               | 70-75                                 |
| 11.141 | Tungsten         | Silver               | 70-75                                 |
| 11.142 | Tungsten         | Gold                 | 70-75                                 |
| 11.143 | Tungsten         | Cobalt               | 75-80                                 |
| 11.144 | Tungsten         | Nickel               | 75-80                                 |
| 11.145 | Tungsten         | Rhodium              | 75-80                                 |
| 11.146 | Tungsten         | Palladium            | 75-80                                 |
| 11.147 | Tungsten         | Platinum             | 75-80                                 |
| 11.148 | Tungsten         | Copper               | 75-80                                 |
| 11.149 | Tungsten         | Silver               | 75-80                                 |
| 11.150 | Tungsten         | Gold                 | 75-80                                 |
| 11.151 | Tungsten         | Cobalt               | 80-85                                 |
| 11.152 | Tungsten         | Nickel               | 80-85                                 |
| 11.153 | Tungsten         | Rhodium              | 80-85                                 |
| 11.154 | Tungsten         | Palladium            | 80-85                                 |
| 11.155 | Tungsten         | Platinum             | 80-85                                 |
| 11.156 | Tungsten         | Copper               | 80-85                                 |
| 11.157 | Tungsten         | Silver               | 80-85                                 |
| 11.158 | Tungsten         | Gold                 | 80-85                                 |
| 1      |                  |                      |                                       |

TABLE 13-continued

| No.    | Refractory metal | Non-refractory metal | Amount of non-refractory metal (wt.%) |
|--------|------------------|----------------------|---------------------------------------|
| 13.014 | Titanium         | Copper               | 5-10                                  |
| 13.015 | Titanium         | Silver               | 5-10                                  |
| 13.016 | Titanium         | Gold                 | 5-10                                  |
| 13.017 | Titanium         | Cobalt               | 10-15                                 |
| 13.018 | Titanium         | Nickel               | 10-15                                 |
| 13.019 | Titanium         | Rhodium              | 10-15                                 |
| 13.020 | Titanium         | Palladium            | 10-15                                 |
| 13.021 | Titanium         | Platinum             | 10-15                                 |
| 13.022 | Titanium         | Copper               | 10-15                                 |
| 13.023 | Titanium         | Silver               | 10-15                                 |
| 13.024 | Titanium         | Gold                 | 10-15                                 |
| 13.025 | Titanium         | Cobalt               | 15-20                                 |
| 13.026 | Titanium         | Nickel               | 15-20                                 |
| 13.027 | Titanium         | Rhodium              | 15-20                                 |
| 13.028 | Titanium         | Palladium            | 15-20                                 |
| 13.029 | Titanium         | Platinum             | 15-20                                 |
| 13.030 | Titanium         | Copper               | 15-20                                 |
| 13.031 | Titanium         | Silver               | 15-20                                 |
| 13.032 | Titanium         | Gold                 | 15-20                                 |
| 13.033 | Titanium         | Cobalt               | 20-25                                 |
| 13.034 | Titanium         | Nickel               | 20-25                                 |
| 13.035 | Titanium         | Rhodium              | 20-25                                 |
| 13.036 | Titanium         | Palladium            | 20-25                                 |
| 13.037 | Titanium         | Platinum             | 20-25                                 |
| 13.038 | Titanium         | Copper               | 20-25                                 |
| 13.039 | Titanium         | Silver               | 20-25                                 |
| 13.040 | Titanium         | Gold                 | 20-25                                 |
| 13.041 | Titanium         | Cobalt               | 25-30                                 |
| 13.042 | Titanium         | Nickel               | 25-30                                 |
| 13.043 | Titanium         | Rhodium              | 25-30                                 |
| 13.044 | Titanium         | Palladium            | 25-30                                 |
| 13.045 | Titanium         | Platinum             | 25-30                                 |
| 13.046 | Titanium         | Copper               | 25-30                                 |
| 13.047 | Titanium         | Silver               | 25-30                                 |
| 13.048 | Titanium         | Gold                 | 25-30                                 |

Table 14: Table 14 consists of 48 pseudo alloys, the refractory metal being niobium and the non-refractory metal and the amount thereof in wt. % being as indicated in Table 1.

TABLE 14

| No.    | Refractory metal | Non-refractory metal | Amount of non-refractory metal (wt.%) |
|--------|------------------|----------------------|---------------------------------------|
| 14.001 | Niobium          | Cobalt               | 2-5                                   |
| 14.002 | Niobium          | Nickel               | 2-5                                   |
| 14.003 | Niobium          | Rhodium              | 2-5                                   |
| 14.004 | Niobium          | Palladium            | 2-5                                   |
| 14.005 | Niobium          | Platinum             | 2-5                                   |
| 14.006 | Niobium          | Copper               | 2-5                                   |
| 14.007 | Niobium          | Silver               | 2-5                                   |
| 14.008 | Niobium          | Gold                 | 2-5                                   |
| 14.009 | Niobium          | Cobalt               | 5-10                                  |
| 14.010 | Niobium          | Nickel               | 5-10                                  |
| 14.011 | Niobium          | Rhodium              | 5-10                                  |
| 14.012 | Niobium          | Palladium            | 5-10                                  |
| 14.013 | Niobium          | Platinum             | 5-10                                  |
| 14.014 | Niobium          | Copper               | 5-10                                  |
| 14.015 | Niobium          | Silver               | 5-10                                  |
| 14.016 | Niobium          | Gold                 | 5-10                                  |
| 14.017 | Niobium          | Cobalt               | 10-15                                 |
| 14.018 | Niobium          | Nickel               | 10-15                                 |
| 14.019 | Niobium          | Rhodium              | 10-15                                 |
| 14.020 | Niobium          | Palladium            | 10-15                                 |
| 14.021 | Niobium          | Platinum             | 10-15                                 |
| 14.022 | Niobium          | Copper               | 10-15                                 |
| 14.023 | Niobium          | Silver               | 10-15                                 |
| 14.024 | Niobium          | Gold                 | 10-15                                 |
| 14.025 | Niobium          | Cobalt               | 15-20                                 |
| 14.026 | Niobium          | Nickel               | 15-20                                 |
| 14.027 | Niobium          | Rhodium              | 15-20                                 |
| 14.028 | Niobium          | Palladium            | 15-20                                 |

TABLE 14-continued

| No.    | Refractory metal | Non-refractory metal | Amount of non-refractory metal (wt.%) |
|--------|------------------|----------------------|---------------------------------------|
| 5      | 14.029           | Niobium              | Platinum                              |
| 10     | 14.030           | Niobium              | Copper                                |
| 14.031 | Niobium          | Silver               | 15-20                                 |
| 14.032 | Niobium          | Gold                 | 15-20                                 |
| 14.033 | Niobium          | Cobalt               | 20-25                                 |
| 14.034 | Niobium          | Nickel               | 20-25                                 |
| 14.035 | Niobium          | Rhodium              | 20-25                                 |
| 14.036 | Niobium          | Palladium            | 20-25                                 |
| 14.037 | Niobium          | Platinum             | 20-25                                 |
| 14.038 | Niobium          | Copper               | 20-25                                 |
| 14.039 | Niobium          | Silver               | 20-25                                 |
| 14.040 | Niobium          | Gold                 | 20-25                                 |
| 14.041 | Niobium          | Cobalt               | 25-30                                 |
| 14.042 | Niobium          | Nickel               | 25-30                                 |
| 14.043 | Niobium          | Rhodium              | 25-30                                 |
| 14.044 | Niobium          | Palladium            | 25-30                                 |
| 14.045 | Niobium          | Platinum             | 25-30                                 |
| 14.046 | Niobium          | Copper               | 25-30                                 |
| 14.047 | Niobium          | Silver               | 25-30                                 |
| 14.048 | Niobium          | Gold                 | 25-30                                 |

Table 15: Table 15 consists of 48 powder mixtures, the refractory metal being niobium and non-refractory metal and the amount thereof in wt. % being as indicated in Table 1.

TABLE 15

| No.    | Refractory metal | Non-refractory metal | Amount of non-refractory metal (wt.%) |
|--------|------------------|----------------------|---------------------------------------|
| 35     | 15.001           | Niobium              | Cobalt                                |
| 15.002 | Niobium          | Nickel               | 2-5                                   |
| 15.003 | Niobium          | Rhodium              | 2-5                                   |
| 15.004 | Niobium          | Palladium            | 2-5                                   |
| 15.005 | Niobium          | Platinum             | 2-5                                   |
| 15.006 | Niobium          | Copper               | 2-5                                   |
| 15.007 | Niobium          | Silver               | 2-5                                   |
| 15.008 | Niobium          | Gold                 | 2-5                                   |
| 15.009 | Niobium          | Cobalt               | 5-10                                  |
| 15.010 | Niobium          | Nickel               | 5-10                                  |
| 15.011 | Niobium          | Rhodium              | 5-10                                  |
| 15.012 | Niobium          | Palladium            | 5-10                                  |
| 15.013 | Niobium          | Platinum             | 5-10                                  |
| 15.014 | Niobium          | Copper               | 5-10                                  |
| 15.015 | Niobium          | Silver               | 5-10                                  |
| 40     | 15.016           | Niobium              | Gold                                  |
| 15.017 | Niobium          | Cobalt               | 10-15                                 |
| 15.018 | Niobium          | Nickel               | 10-15                                 |
| 15.019 | Niobium          | Rhodium              | 10-15                                 |
| 15.020 | Niobium          | Palladium            | 10-15                                 |
| 15.021 | Niobium          | Platinum             | 10-15                                 |
| 15.022 | Niobium          | Copper               | 10-15                                 |
| 50     | 15.023           | Niobium              | Silver                                |
| 15.024 | Niobium          | Gold                 | 10-15                                 |
| 15.025 | Niobium          | Cobalt               | 15-20                                 |
| 15.026 | Niobium          | Nickel               | 15-20                                 |
| 15.027 | Niobium          | Rhodium              | 15-20                                 |
| 15.028 | Niobium          | Palladium            | 15-20                                 |
| 55     | 15.029           | Niobium              | Platinum                              |
| 15.030 | Niobium          | Copper               | 15-20                                 |
| 15.031 | Niobium          | Silver               | 15-20                                 |
| 15.032 | Niobium          | Gold                 | 15-20                                 |
| 15.033 | Niobium          | Cobalt               | 20-25                                 |
| 15.034 | Niobium          | Nickel               | 20-25                                 |
| 15.035 | Niobium          | Rhodium              | 20-25                                 |
| 60     | 15.036           | Niobium              | Palladium                             |
| 15.037 | Niobium          | Platinum             | 20-25                                 |
| 15.038 | Niobium          | Copper               | 20-25                                 |
| 15.039 | Niobium          | Silver               | 20-25                                 |
| 65     | 15.040           | Niobium              | Gold                                  |
| 15.041 | Niobium          | Cobalt               | 25-30                                 |
| 15.042 | Niobium          | Nickel               | 25-30                                 |
| 15.043 | Niobium          | Rhodium              | 25-30                                 |

TABLE 15-continued

| No.    | Refractory metal | Non-refractory metal | Amount of non-refractory metal (wt.%) |
|--------|------------------|----------------------|---------------------------------------|
| 15.044 | Niobium          | Palladium            | 25-30                                 |
| 15.045 | Niobium          | Platinum             | 25-30                                 |
| 15.046 | Niobium          | Copper               | 25-30                                 |
| 15.047 | Niobium          | Silver               | 25-30                                 |
| 15.048 | Niobium          | Gold                 | 25-30                                 |

Table 17: Table 17 consists of 20 alloys, pseudo alloys and powder mixtures according to Table 16, component 1 being present in an amount of 2-5 wt. %, component 2 being present in an amount ad 100 wt. % and the individual partners in the mixture being as listed in Table 16.

TABLE 17

| Component 1 | Amount of component 1 | Component 2 | Amount of component 2 |
|-------------|-----------------------|-------------|-----------------------|
| 17.001      | Nb                    | 2-5 wt. %   | Ta ad 100 wt. %       |
| 17.002      | Nb                    | 2-5 wt. %   | W ad 100 wt. %        |
| 17.003      | Nb                    | 2-5 wt. %   | Mo ad 100 wt. %       |
| 17.004      | Nb                    | 2-5 wt. %   | Ti ad 100 wt. %       |
| 17.005      | Ta                    | 2-5 wt. %   | Nb ad 100 wt. %       |
| 17.006      | Ta                    | 2-5 wt. %   | W ad 100 wt. %        |
| 17.007      | Ta                    | 2-5 wt. %   | Mo ad 100 wt. %       |
| 17.008      | Ta                    | 2-5 wt. %   | Ti ad 100 wt. %       |
| 17.009      | W                     | 2-5 wt. %   | Ta ad 100 wt. %       |
| 17.010      | W                     | 2-5 wt. %   | Nb ad 100 wt. %       |
| 17.011      | W                     | 2-5 wt. %   | Mo ad 100 wt. %       |
| 17.012      | W                     | 2-5 wt. %   | Ti ad 100 wt. %       |
| 17.013      | Mo                    | 2-5 wt. %   | Ta ad 100 wt. %       |
| 17.014      | Mo                    | 2-5 wt. %   | Nb ad 100 wt. %       |
| 17.015      | Mo                    | 2-5 wt. %   | W ad 100 wt. %        |
| 17.016      | Mo                    | 2-5 wt. %   | Ti ad 100 wt. %       |
| 17.017      | Ti                    | 2-5 wt. %   | Ta ad 100 wt. %       |
| 17.018      | Ti                    | 2-5 wt. %   | Nb ad 100 wt. %       |
| 17.019      | Ti                    | 2-5 wt. %   | W ad 100 wt. %        |
| 17.020      | Ti                    | 2-5 wt. %   | Mo ad 100 wt. %       |

Table 18: Table 18 consists of 20 alloys, pseudo alloys and powder mixtures according to Table 16, component 1 being present in an amount of 5-10 wt. %, component 2 being present in an amount ad 100 wt. % and the individual partners in the mixture being listed in Table 16.

TABLE 18

| Component 1 | Amount of component 1 | Component 2 | Amount of component 2 |
|-------------|-----------------------|-------------|-----------------------|
| 18.001      | Nb                    | 5-10 wt. %  | Ta ad 100 wt. %       |
| 18.002      | Nb                    | 5-10 wt. %  | W ad 100 wt. %        |
| 18.003      | Nb                    | 5-10 wt. %  | Mo ad 100 wt. %       |
| 18.004      | Nb                    | 5-10 wt. %  | Ti ad 100 wt. %       |
| 18.005      | Ta                    | 5-10 wt. %  | Nb ad 100 wt. %       |
| 18.006      | Ta                    | 5-10 wt. %  | W ad 100 wt. %        |
| 18.007      | Ta                    | 5-10 wt. %  | Mo ad 100 wt. %       |
| 18.008      | Ta                    | 5-10 wt. %  | Ti ad 100 wt. %       |
| 18.009      | W                     | 5-10 wt. %  | Ta ad 100 wt. %       |
| 18.010      | W                     | 5-10 wt. %  | Nb ad 100 wt. %       |
| 18.011      | W                     | 5-10 wt. %  | Mo ad 100 wt. %       |
| 18.012      | W                     | 5-10 wt. %  | Ti ad 100 wt. %       |
| 18.013      | Mo                    | 5-10 wt. %  | Ta ad 100 wt. %       |
| 18.014      | Mo                    | 5-10 wt. %  | Nb ad 100 wt. %       |
| 18.015      | Mo                    | 5-10 wt. %  | W ad 100 wt. %        |
| 18.016      | Mo                    | 5-10 wt. %  | Ti ad 100 wt. %       |
| 18.017      | Ti                    | 5-10 wt. %  | Ta ad 100 wt. %       |
| 18.018      | Ti                    | 5-10 wt. %  | Nb ad 100 wt. %       |
| 18.019      | Ti                    | 5-10 wt. %  | W ad 100 wt. %        |
| 18.020      | Ti                    | 5-10 wt. %  | Mo ad 100 wt. %       |

Table 19: Table 19 consists of 20 alloys, pseudo alloys and powder mixtures according to Table 16, component 1 being present in an amount of 10-15 wt. %, component 2 being present in an amount ad 100 wt. % and the individual partners in the mixture being as listed in Table 16.

TABLE 19

| Component 1 | Amount of component 1 | Component 2 | Amount of component 2 |
|-------------|-----------------------|-------------|-----------------------|
| 19.001      | Nb                    | 10-15 wt. % | Ta ad 100 wt. %       |
| 19.002      | Nb                    | 10-15 wt. % | W ad 100 wt. %        |
| 19.003      | Nb                    | 10-15 wt. % | Mo ad 100 wt. %       |
| 19.004      | Nb                    | 10-15 wt. % | Ti ad 100 wt. %       |
| 19.005      | Ta                    | 10-15 wt. % | Nb ad 100 wt. %       |
| 19.006      | Ta                    | 10-15 wt. % | W ad 100 wt. %        |
| 19.007      | Ta                    | 10-15 wt. % | Mo ad 100 wt. %       |
| 19.008      | Ta                    | 10-15 wt. % | Ti ad 100 wt. %       |
| 19.009      | W                     | 10-15 wt. % | Ta ad 100 wt. %       |
| 19.010      | W                     | 10-15 wt. % | Nb ad 100 wt. %       |
| 19.011      | W                     | 10-15 wt. % | Mo ad 100 wt. %       |
| 19.012      | W                     | 10-15 wt. % | Ti ad 100 wt. %       |
| 19.013      | Mo                    | 10-15 wt. % | Ta ad 100 wt. %       |
| 19.014      | Mo                    | 10-15 wt. % | Nb ad 100 wt. %       |
| 19.015      | Mo                    | 10-15 wt. % | W ad 100 wt. %        |
| 19.016      | Mo                    | 10-15 wt. % | Ti ad 100 wt. %       |
| 19.017      | Ti                    | 10-15 wt. % | Ta ad 100 wt. %       |
| 19.018      | Ti                    | 10-15 wt. % | Nb ad 100 wt. %       |
| 19.019      | Ti                    | 10-15 wt. % | W ad 100 wt. %        |
| 19.020      | Ti                    | 10-15 wt. % | Mo ad 100 wt. %       |

Table 20: Table 20 consists of 20 alloys, pseudo alloys and powder mixtures according to Table 16, component 1 being present in an amount of 15-20 wt. %, component 2 being present in an amount ad 100 wt. % and the individual partners in the mixture being as listed in Table 16.

TABLE 20

| Component 1 | Amount of component 1 | Component 2 | Amount of component 2 |
|-------------|-----------------------|-------------|-----------------------|
| 20.001      | Nb                    | 15-20 wt. % | Ta ad 100 wt. %       |
| 20.002      | Nb                    | 15-20 wt. % | W ad 100 wt. %        |
| 20.003      | Nb                    | 15-20 wt. % | Mo ad 100 wt. %       |
| 20.004      | Nb                    | 15-20 wt. % | Ti ad 100 wt. %       |
| 20.005      | Ta                    | 15-20 wt. % | Nb ad 100 wt. %       |
| 20.006      | Ta                    | 15-20 wt. % | W ad 100 wt. %        |
| 20.007      | Ta                    | 15-20 wt. % | Mo ad 100 wt. %       |
| 20.008      | Ta                    | 15-20 wt. % | Ti ad 100 wt. %       |
| 20.009      | W                     | 15-20 wt. % | Ta ad 100 wt. %       |
| 20.010      | W                     | 15-20 wt. % | Nb ad 100 wt. %       |
| 20.011      | W                     | 15-20 wt. % | Mo ad 100 wt. %       |
| 20.012      | W                     | 15-20 wt. % | Ti ad 100 wt. %       |
| 20.013      | Mo                    | 15-20 wt. % | Ta ad 100 wt. %       |
| 20.014      | Mo                    | 15-20 wt. % | Nb ad 100 wt. %       |
| 20.015      | Mo                    | 15-20 wt. % | W ad 100 wt. %        |
| 20.016      | Mo                    | 15-20 wt. % | Ti ad 100 wt. %       |
| 20.017      | Ti                    | 15-20 wt. % | Ta ad 100 wt. %       |
| 20.018      | Ti                    | 15-20 wt. % | Nb ad 100 wt. %       |
| 20.019      | Ti                    | 15-20 wt. % | W ad 100 wt. %        |
| 20.020      | Ti                    | 15-20 wt. % | Mo ad 100 wt. %       |

Table 21: Table 21 consists of 20 alloys, pseudo alloys and powder mixtures according to Table 16, component 1 being present in an amount of 20-25 wt. %, component 2 being present in an amount ad 100 wt. % and the individual partners in the mixture being as listed in Table 16.

TABLE 21

| Component 1 | Amount of component 1 | Component 2 | Amount of component 2 |
|-------------|-----------------------|-------------|-----------------------|
| 21.001      | Nb                    | 20-25 wt. % | Ta                    |
| 21.002      | Nb                    | 20-25 wt. % | W                     |
| 21.003      | Nb                    | 20-25 wt. % | Mo                    |
| 21.004      | Nb                    | 20-25 wt. % | Ti                    |
| 21.005      | Ta                    | 20-25 wt. % | Nb                    |
| 21.006      | Ta                    | 20-25 wt. % | W                     |
| 21.007      | Ta                    | 20-25 wt. % | Mo                    |
| 21.008      | Ta                    | 20-25 wt. % | Ti                    |
| 21.009      | W                     | 20-25 wt. % | Ta                    |
| 21.010      | W                     | 20-25 wt. % | Nb                    |
| 21.011      | W                     | 20-25 wt. % | Mo                    |
| 21.012      | W                     | 20-25 wt. % | Ti                    |
| 21.013      | Mo                    | 20-25 wt. % | Ta                    |
| 21.014      | Mo                    | 20-25 wt. % | Nb                    |
| 21.015      | Mo                    | 20-25 wt. % | W                     |
| 21.016      | Mo                    | 20-25 wt. % | Ti                    |
| 21.017      | Ti                    | 20-25 wt. % | Ta                    |
| 21.018      | Ti                    | 20-25 wt. % | Nb                    |
| 21.019      | Ti                    | 20-25 wt. % | W                     |
| 21.020      | Ti                    | 20-25 wt. % | Mo                    |

Table 22: Table 22 consists of 20 alloys, pseudo alloys and powder mixtures according to Table 16, component 1 being present in an amount of 25-30 wt. %, component 2 being present in an amount ad 100 wt. % and the individual partners in the mixture being as listed in Table 16.

TABLE 22

| Component 1 | Amount of component 1 | Component 2 | Amount of component 2 |
|-------------|-----------------------|-------------|-----------------------|
| 22.001      | Nb                    | 25-30 wt. % | Ta                    |
| 22.002      | Nb                    | 25-30 wt. % | W                     |
| 22.003      | Nb                    | 25-30 wt. % | Mo                    |
| 22.004      | Nb                    | 25-30 wt. % | Ti                    |
| 22.005      | Ta                    | 25-30 wt. % | Nb                    |
| 22.006      | Ta                    | 25-30 wt. % | W                     |
| 22.007      | Ta                    | 25-30 wt. % | Mo                    |
| 22.008      | Ta                    | 25-30 wt. % | Ti                    |
| 22.009      | W                     | 25-30 wt. % | Ta                    |
| 22.010      | W                     | 25-30 wt. % | Nb                    |
| 22.011      | W                     | 25-30 wt. % | Mo                    |
| 22.012      | W                     | 25-30 wt. % | Ti                    |
| 22.013      | Mo                    | 25-30 wt. % | Ta                    |
| 22.014      | Mo                    | 25-30 wt. % | Nb                    |
| 22.015      | Mo                    | 25-30 wt. % | W                     |
| 22.016      | Mo                    | 25-30 wt. % | Ti                    |
| 22.017      | Ti                    | 25-30 wt. % | Ta                    |
| 22.018      | Ti                    | 25-30 wt. % | Nb                    |
| 22.019      | Ti                    | 25-30 wt. % | W                     |
| 22.020      | Ti                    | 25-30 wt. % | Mo                    |

Table 23: Table 23 consists of 20 alloys, pseudo alloys and powder mixtures according to Table 16, component 1 being present in an amount of 30-35 wt. %, component 2 being present in an amount ad 100 wt. % and the individual partners in the mixture being as listed in Table 16.

TABLE 23

| Component 1 | Amount of component 1 | Component 2 | Amount of component 2 |
|-------------|-----------------------|-------------|-----------------------|
| 23.001      | Nb                    | 30-35 wt. % | Ta                    |
| 23.002      | Nb                    | 30-35 wt. % | W                     |
| 23.003      | Nb                    | 30-35 wt. % | Mo                    |
| 23.004      | Nb                    | 30-35 wt. % | Ti                    |
| 23.005      | Ta                    | 30-35 wt. % | Nb                    |
| 23.006      | Ta                    | 30-35 wt. % | W                     |
| 23.007      | Ta                    | 30-35 wt. % | Mo                    |
| 23.008      | Ta                    | 30-35 wt. % | Ti                    |

TABLE 23-continued

| Component 1 | Amount of component 1 | Component 2 | Amount of component 2 |
|-------------|-----------------------|-------------|-----------------------|
| 5           | 23.009                | W           | 30-35 wt. %           |
|             | 23.010                | W           | 30-35 wt. %           |
|             | 23.011                | W           | 30-35 wt. %           |
|             | 23.012                | W           | 30-35 wt. %           |
|             | 23.013                | Mo          | 30-35 wt. %           |
|             | 23.014                | Mo          | 30-35 wt. %           |
| 10          | 23.015                | Mo          | 30-35 wt. %           |
|             | 23.016                | Mo          | 30-35 wt. %           |
|             | 23.017                | Ti          | 30-35 wt. %           |
|             | 23.018                | Ti          | 30-35 wt. %           |
|             | 23.019                | Ti          | 30-35 wt. %           |
|             | 23.020                | Ti          | 30-35 wt. %           |

Table 24: Table 24 consists of 20 alloys, pseudo alloys and powder mixtures according to Table 16, component 1 being present in an amount of 35-40 wt. %, component 2 being present in an amount ad 100 wt. % and the individual partners in the mixture being as listed in Table 16.

TABLE 24

| Component 1 | Amount of component 1 | Component 2 | Amount of component 2 |
|-------------|-----------------------|-------------|-----------------------|
| 25          | 24.001                | Nb          | 35-40 wt. %           |
|             | 24.002                | Nb          | 35-40 wt. %           |
|             | 24.003                | Nb          | 35-40 wt. %           |
|             | 24.004                | Nb          | 35-40 wt. %           |
|             | 24.005                | Ta          | 35-40 wt. %           |
| 30          | 24.006                | Ta          | 35-40 wt. %           |
|             | 24.007                | Ta          | 35-40 wt. %           |
|             | 24.008                | Ta          | 35-40 wt. %           |
|             | 24.009                | W           | 35-40 wt. %           |
|             | 24.010                | W           | 35-40 wt. %           |
| 35          | 24.011                | W           | 35-40 wt. %           |
|             | 24.012                | W           | 35-40 wt. %           |
|             | 24.013                | Mo          | 35-40 wt. %           |
|             | 24.014                | Mo          | 35-40 wt. %           |
|             | 24.015                | Mo          | 35-40 wt. %           |
|             | 24.016                | Mo          | 35-40 wt. %           |
| 40          | 24.017                | Ti          | 35-40 wt. %           |
|             | 24.018                | Ti          | 35-40 wt. %           |
|             | 24.019                | Ti          | 35-40 wt. %           |
|             | 24.020                | Ti          | 35-40 wt. %           |

Table 25: Table 25 consists of 20 alloys, pseudo alloys and powder mixtures according to Table 16, component 1 being present in an amount of 40-45 wt. %, component 2 being present in an amount ad 100 wt. % and the individual partners in the mixture being as listed in Table 16.

TABLE 25

| Component 1 | Amount of component 1 | Component 2 | Amount of component 2 |
|-------------|-----------------------|-------------|-----------------------|
| 50          | 25.001                | Nb          | 40-45 wt. %           |
|             | 25.002                | Nb          | 40-45 wt. %           |
|             | 25.003                | Nb          | 40-45 wt. %           |
|             | 25.004                | Nb          | 40-45 wt. %           |
|             | 25.005                | Ta          | 40-45 wt. %           |
| 55          | 25.006                | Ta          | 40-45 wt. %           |
|             | 25.007                | Ta          | 40-45 wt. %           |
|             | 25.008                | Ta          | 40-45 wt. %           |
| 60          | 25.009                | W           | 40-45 wt. %           |
|             | 25.010                | W           | 40-45 wt. %           |
|             | 25.011                | W           | 40-45 wt. %           |
|             | 25.012                | W           | 40-45 wt. %           |
|             | 25.013                | Mo          | 40-45 wt. %           |
| 65          | 25.014                | Mo          | 40-45 wt. %           |
|             | 25.015                | Mo          | 40-45 wt. %           |
|             | 25.016                | Mo          | 40-45 wt. %           |

TABLE 25-continued

| Component 1 | Amount of component 1 | Component 2 | Amount of component 2 |
|-------------|-----------------------|-------------|-----------------------|
| 25.017      | Ti                    | 40-45 wt. % | Ta                    |
| 25.018      | Ti                    | 40-45 wt. % | Nb                    |
| 25.019      | Ti                    | 40-45 wt. % | W                     |
| 25.020      | Ti                    | 40-45 wt. % | Mo                    |

Table 26: Table 26 consists of 20 alloys, pseudo alloys and powder mixtures according to Table 16, component 1 being present in an amount of 45-50 wt. %, component 2 being present in an amount ad 100 wt. % and the individual partners in the mixture being as listed in Table 16.

TABLE 26

| Component 1 | Amount of component 1 | Component 2 | Amount of component 2 |
|-------------|-----------------------|-------------|-----------------------|
| 26.001      | Nb                    | 45-50 wt. % | Ta                    |
| 26.002      | Nb                    | 45-50 wt. % | W                     |
| 26.003      | Nb                    | 45-50 wt. % | Mo                    |
| 26.004      | Nb                    | 45-50 wt. % | Ti                    |
| 26.005      | Ta                    | 45-50 wt. % | Nb                    |
| 26.006      | Ta                    | 45-50 wt. % | W                     |
| 26.007      | Ta                    | 45-50 wt. % | Mo                    |
| 26.008      | Ta                    | 45-50 wt. % | Ti                    |
| 26.009      | W                     | 45-50 wt. % | Ta                    |
| 26.010      | W                     | 45-50 wt. % | Nb                    |
| 26.011      | W                     | 45-50 wt. % | Mo                    |
| 26.012      | W                     | 45-50 wt. % | Ti                    |
| 26.013      | Mo                    | 45-50 wt. % | Ta                    |
| 26.014      | Mo                    | 45-50 wt. % | Nb                    |
| 26.015      | Mo                    | 45-50 wt. % | W                     |
| 26.016      | Mo                    | 45-50 wt. % | Ti                    |
| 26.017      | Ti                    | 45-50 wt. % | Ta                    |
| 26.018      | Ti                    | 45-50 wt. % | Nb                    |
| 26.019      | Ti                    | 45-50 wt. % | W                     |
| 26.020      | Ti                    | 45-50 wt. % | Mo                    |

Table 27: Table 27 consists of 20 alloys, pseudo alloys and powder mixtures according to Table 16, component 1 being present in an amount of 50-55 wt. %, component 2 being present in an amount ad 100 wt. % and the individual partners in the mixture being as listed in Table 16.

TABLE 27

| Component 1 | Amount of component 1 | Component 2 | Amount of component 2 |
|-------------|-----------------------|-------------|-----------------------|
| 27.001      | Nb                    | 50-55 wt. % | Ta                    |
| 27.002      | Nb                    | 50-55 wt. % | W                     |
| 27.003      | Nb                    | 50-55 wt. % | Mo                    |
| 27.004      | Nb                    | 50-55 wt. % | Ti                    |
| 27.005      | Ta                    | 50-55 wt. % | Nb                    |
| 27.006      | Ta                    | 50-55 wt. % | W                     |
| 27.007      | Ta                    | 50-55 wt. % | Mo                    |
| 27.008      | Ta                    | 50-55 wt. % | Ti                    |
| 27.009      | W                     | 50-55 wt. % | Ta                    |
| 27.010      | W                     | 50-55 wt. % | Nb                    |
| 27.011      | W                     | 50-55 wt. % | Mo                    |
| 27.012      | W                     | 50-55 wt. % | Ti                    |
| 27.013      | Mo                    | 50-55 wt. % | Ta                    |
| 27.014      | Mo                    | 50-55 wt. % | Nb                    |
| 27.015      | Mo                    | 50-55 wt. % | W                     |
| 27.016      | Mo                    | 50-55 wt. % | Ti                    |
| 27.017      | Ti                    | 50-55 wt. % | Ta                    |
| 27.018      | Ti                    | 50-55 wt. % | Nb                    |
| 27.019      | Ti                    | 50-55 wt. % | W                     |
| 27.020      | Ti                    | 50-55 wt. % | Mo                    |

Table 28: Table 28 consists of 20 alloys, pseudo alloys and powder mixtures according to Table 16, component 1 being present in an amount of 55-60 wt. %, component 2 being

present in an amount ad 100 wt. % and the individual partners in the mixture being as listed in Table 16.

TABLE 28

| Component 1 | Amount of component 1 | Component 2 | Amount of component 2 |
|-------------|-----------------------|-------------|-----------------------|
| 28.001      | Nb                    | 55-60 wt. % | Ta                    |
| 28.002      | Nb                    | 55-60 wt. % | W                     |
| 28.003      | Nb                    | 55-60 wt. % | Mo                    |
| 28.004      | Nb                    | 55-60 wt. % | Ti                    |
| 28.005      | Ta                    | 55-60 wt. % | Nb                    |
| 28.006      | Ta                    | 55-60 wt. % | W                     |
| 28.007      | Ta                    | 55-60 wt. % | Mo                    |
| 28.008      | Ta                    | 55-60 wt. % | Ti                    |
| 28.009      | W                     | 55-60 wt. % | Ta                    |
| 28.010      | W                     | 55-60 wt. % | Nb                    |
| 28.011      | W                     | 55-60 wt. % | Mo                    |
| 28.012      | W                     | 55-60 wt. % | Ti                    |
| 28.013      | Mo                    | 55-60 wt. % | Ta                    |
| 28.014      | Mo                    | 55-60 wt. % | Nb                    |
| 28.015      | Mo                    | 55-60 wt. % | W                     |
| 28.016      | Mo                    | 55-60 wt. % | Ti                    |
| 28.017      | Ti                    | 55-60 wt. % | Ta                    |
| 28.018      | Ti                    | 55-60 wt. % | Nb                    |
| 28.019      | Ti                    | 55-60 wt. % | W                     |
| 28.020      | Ti                    | 55-60 wt. % | Mo                    |

Also suitable for use in the methods according to the invention are metal powders which consist of alloys, pseudo alloys and powder mixtures of different refractory metals with one another.

For example, alloys of molybdenum and titanium in a ratio of 50:50 atomic percent or alloys of tungsten and titanium in an amount of about 90:10 wt. % are known and are suitable for use in the methods according to the invention. In principle, however, all alloys of the refractory metals with one another are suitable for use in the methods according to the invention.

Binary alloys, pseudo alloys and powder mixtures of refractory metals that are suitable for the methods according to the invention are listed in Tables 16 to 36. Individual materials are designated with the number of the table followed by the number of the combination of components as in Table 16. For example, material 22.005 is a material described in Table 22, the precise composition being defined by the refractory metals, which are listed in Table 16, position no. 5, and the amount as listed in Table 22.

| Component 1 | Component 2 |
|-------------|-------------|
| 16.001      | Nb          |
| 16.002      | W           |
| 16.003      | Mo          |
| 16.004      | Ti          |
| 16.005      | Nb          |
| 16.006      | W           |
| 16.007      | Mo          |
| 16.008      | Ti          |
| 16.009      | Ta          |
| 16.010      | Nb          |
| 16.011      | Mo          |
| 16.012      | Ti          |
| 16.013      | Ta          |
| 16.014      | Nb          |
| 16.015      | W           |
| 16.016      | Ti          |
| 16.017      | Ta          |
| 16.018      | Nb          |
| 16.019      | W           |
| 16.020      | Mo          |

Table 29: Table 29 consists of 20 alloys, pseudo alloys and powder mixtures according to Table 16, component 1 being

present in an amount of 60-65 wt. %, component 2 being present in an amount ad 100 wt. % and the individual partners in the mixture being as listed in Table 16.

TABLE 29

|        | Component 1 | Amount of component 1 | Component 2 | Amount of component 2 |
|--------|-------------|-----------------------|-------------|-----------------------|
| 29.001 | Nb          | 60-65 wt. %           | Ta          | ad 100 wt. %          |
| 29.002 | Nb          | 60-65 wt. %           | W           | ad 100 wt. %          |
| 29.003 | Nb          | 60-65 wt. %           | Mo          | ad 100 wt. %          |
| 29.004 | Nb          | 60-65 wt. %           | Ti          | ad 100 wt. %          |
| 29.005 | Ta          | 60-65 wt. %           | Nb          | ad 100 wt. %          |
| 29.006 | Ta          | 60-65 wt. %           | W           | ad 100 wt. %          |
| 29.007 | Ta          | 60-65 wt. %           | Mo          | ad 100 wt. %          |
| 29.008 | Ta          | 60-65 wt. %           | Ti          | ad 100 wt. %          |
| 29.009 | W           | 60-65 wt. %           | Ta          | ad 100 wt. %          |
| 29.010 | W           | 60-65 wt. %           | Nb          | ad 100 wt. %          |
| 29.011 | W           | 60-65 wt. %           | Mo          | ad 100 wt. %          |
| 29.012 | W           | 60-65 wt. %           | Ti          | ad 100 wt. %          |
| 29.013 | Mo          | 60-65 wt. %           | Ta          | ad 100 wt. %          |
| 29.014 | Mo          | 60-65 wt. %           | Nb          | ad 100 wt. %          |
| 29.015 | Mo          | 60-65 wt. %           | W           | ad 100 wt. %          |
| 29.016 | Mo          | 60-65 wt. %           | Ti          | ad 100 wt. %          |
| 29.017 | Ti          | 60-65 wt. %           | Ta          | ad 100 wt. %          |
| 29.018 | Ti          | 60-65 wt. %           | Nb          | ad 100 wt. %          |
| 29.019 | Ti          | 60-65 wt. %           | W           | ad 100 wt. %          |
| 29.020 | Ti          | 60-65 wt. %           | Mo          | ad 100 wt. %          |

Table 30: Table 30 consists of 20 alloys, pseudo alloys and powder mixtures according to Table 16, component 1 being present in an amount of 65-70 wt. %, component 2 being present in an amount ad 100 wt. % and the individual partners in the mixture being as listed in Table 16.

TABLE 30

|        | Component 1 | Amount of component 1 | Component 2 | Amount of component 2 |
|--------|-------------|-----------------------|-------------|-----------------------|
| 30.001 | Nb          | 65-70 wt. %           | Ta          | ad 100 wt. %          |
| 30.002 | Nb          | 65-70 wt. %           | W           | ad 100 wt. %          |
| 30.003 | Nb          | 65-70 wt. %           | Mo          | ad 100 wt. %          |
| 30.004 | Nb          | 65-70 wt. %           | Ti          | ad 100 wt. %          |
| 30.005 | Ta          | 65-70 wt. %           | Nb          | ad 100 wt. %          |
| 30.006 | Ta          | 65-70 wt. %           | W           | ad 100 wt. %          |
| 30.007 | Ta          | 65-70 wt. %           | Mo          | ad 100 wt. %          |
| 30.008 | Ta          | 65-70 wt. %           | Ti          | ad 100 wt. %          |
| 30.009 | W           | 65-70 wt. %           | Ta          | ad 100 wt. %          |
| 30.010 | W           | 65-70 wt. %           | Nb          | ad 100 wt. %          |
| 30.011 | W           | 65-70 wt. %           | Mo          | ad 100 wt. %          |
| 30.012 | W           | 65-70 wt. %           | Ti          | ad 100 wt. %          |
| 30.013 | Mo          | 65-70 wt. %           | Ta          | ad 100 wt. %          |
| 30.014 | Mo          | 65-70 wt. %           | Nb          | ad 100 wt. %          |
| 30.015 | Mo          | 65-70 wt. %           | W           | ad 100 wt. %          |
| 30.016 | Mo          | 65-70 wt. %           | Ti          | ad 100 wt. %          |
| 30.017 | Ti          | 65-70 wt. %           | Ta          | ad 100 wt. %          |
| 30.018 | Ti          | 65-70 wt. %           | Nb          | ad 100 wt. %          |
| 30.019 | Ti          | 65-70 wt. %           | W           | ad 100 wt. %          |
| 30.020 | Ti          | 65-70 wt. %           | Mo          | ad 100 wt. %          |

Table 31: Table 31 consists of 20 alloys, pseudo alloys and powder mixtures according to Table 16, component 1 being present in an amount of 70-75 wt. %, component 2 being present in an amount ad 100 wt. % and the individual partners in the mixture being as listed in Table 16.

TABLE 31

|        | Component 1 | Amount of component 1 | Component 2 | Amount of component 2 |
|--------|-------------|-----------------------|-------------|-----------------------|
| 31.001 | Nb          | 70-75 wt. %           | Ta          | ad 100 wt. %          |
| 31.002 | Nb          | 70-75 wt. %           | W           | ad 100 wt. %          |
| 31.003 | Nb          | 70-75 wt. %           | Mo          | ad 100 wt. %          |

TABLE 31-continued

|    | Component 1 | Amount of component 1 | Component 2 | Amount of component 2 |              |
|----|-------------|-----------------------|-------------|-----------------------|--------------|
| 5  | 31.004      | Nb                    | 70-75 wt. % | Ti                    | ad 100 wt. % |
|    | 31.005      | Ta                    | 70-75 wt. % | Nb                    | ad 100 wt. % |
|    | 31.006      | Ta                    | 70-75 wt. % | W                     | ad 100 wt. % |
|    | 31.007      | Ta                    | 70-75 wt. % | Mo                    | ad 100 wt. % |
|    | 31.008      | Ta                    | 70-75 wt. % | Ti                    | ad 100 wt. % |
|    | 31.009      | W                     | 70-75 wt. % | Ta                    | ad 100 wt. % |
|    | 31.010      | W                     | 70-75 wt. % | Nb                    | ad 100 wt. % |
|    | 31.011      | W                     | 70-75 wt. % | Mo                    | ad 100 wt. % |
|    | 31.012      | W                     | 70-75 wt. % | Ti                    | ad 100 wt. % |
|    | 31.013      | Mo                    | 70-75 wt. % | Ta                    | ad 100 wt. % |
| 10 | 31.014      | Mo                    | 70-75 wt. % | Nb                    | ad 100 wt. % |
|    | 31.015      | Mo                    | 70-75 wt. % | W                     | ad 100 wt. % |
|    | 31.016      | Mo                    | 70-75 wt. % | Ti                    | ad 100 wt. % |
|    | 31.017      | Ti                    | 70-75 wt. % | Ta                    | ad 100 wt. % |
|    | 31.018      | Ti                    | 70-75 wt. % | Nb                    | ad 100 wt. % |
|    | 31.019      | Ti                    | 70-75 wt. % | W                     | ad 100 wt. % |
|    | 31.020      | Ti                    | 70-75 wt. % | Mo                    | ad 100 wt. % |

20 Table 32: Table 32 consists of 20 alloys, pseudo alloys and powder mixtures according to Table 16, component 1 being present in an amount of 75-80 wt. %, component 2 being present in an amount ad 100 wt. % and the individual partners in the mixture being as listed in Table 16.

TABLE 32

|    | Component 1 | Amount of component 1 | Component 2 | Amount of component 2 |              |
|----|-------------|-----------------------|-------------|-----------------------|--------------|
| 30 | 32.001      | Nb                    | 75-80 wt. % | Ta                    | ad 100 wt. % |
|    | 32.002      | Nb                    | 75-80 wt. % | W                     | ad 100 wt. % |
|    | 32.003      | Nb                    | 75-80 wt. % | Mo                    | ad 100 wt. % |
|    | 32.004      | Nb                    | 75-80 wt. % | Ti                    | ad 100 wt. % |
|    | 32.005      | Ta                    | 75-80 wt. % | Nb                    | ad 100 wt. % |
|    | 32.006      | Ta                    | 75-80 wt. % | W                     | ad 100 wt. % |
|    | 32.007      | Ta                    | 75-80 wt. % | Mo                    | ad 100 wt. % |
|    | 32.008      | Ta                    | 75-80 wt. % | Ti                    | ad 100 wt. % |
|    | 32.009      | W                     | 75-80 wt. % | Ta                    | ad 100 wt. % |
|    | 32.010      | W                     | 75-80 wt. % | Nb                    | ad 100 wt. % |
| 35 | 32.011      | W                     | 75-80 wt. % | Mo                    | ad 100 wt. % |
|    | 32.012      | W                     | 75-80 wt. % | Ti                    | ad 100 wt. % |
|    | 32.013      | Mo                    | 75-80 wt. % | Ta                    | ad 100 wt. % |
|    | 32.014      | Mo                    | 75-80 wt. % | Nb                    | ad 100 wt. % |
|    | 32.015      | Mo                    | 75-80 wt. % | W                     | ad 100 wt. % |
|    | 32.016      | Mo                    | 75-80 wt. % | Ti                    | ad 100 wt. % |
|    | 32.017      | Ti                    | 75-80 wt. % | Ta                    | ad 100 wt. % |
|    | 32.018      | Ti                    | 75-80 wt. % | Nb                    | ad 100 wt. % |
|    | 32.019      | Ti                    | 75-80 wt. % | W                     | ad 100 wt. % |
|    | 32.020      | Ti                    | 75-80 wt. % | Mo                    | ad 100 wt. % |

50 Table 33: Table 33 consists of 20 alloys, pseudo alloys and powder mixtures according to Table 16, component 1 being present in an amount of 80-85 wt. %, component 2 being present in an amount ad 100 wt. % and the individual partners in the mixture being as listed in Table 16.

TABLE 33

|    | Component 1 | Amount of component 1 | Component 2 | Amount of component 2 |              |
|----|-------------|-----------------------|-------------|-----------------------|--------------|
| 55 | 33.001      | Nb                    | 80-85 wt. % | Ta                    | ad 100 wt. % |
|    | 33.002      | Nb                    | 80-85 wt. % | W                     | ad 100 wt. % |
|    | 33.003      | Nb                    | 80-85 wt. % | Mo                    | ad 100 wt. % |
|    | 33.004      | Nb                    | 80-85 wt. % | Ti                    | ad 100 wt. % |
|    | 33.005      | Ta                    | 80-85 wt. % | Nb                    | ad 100 wt. % |
|    | 33.006      | Ta                    | 80-85 wt. % | W                     | ad 100 wt. % |
|    | 33.007      | Ta                    | 80-85 wt. % | Mo                    | ad 100 wt. % |
|    | 33.008      | Ta                    | 80-85 wt. % | Ti                    | ad 100 wt. % |
|    | 33.009      | W                     | 80-85 wt. % | Ta                    | ad 100 wt. % |
|    | 33.010      | W                     | 80-85 wt. % | Nb                    | ad 100 wt. % |
| 60 | 33.011      | W                     | 80-85 wt. % | Mo                    | ad 100 wt. % |
|    | 33.012      | Ti                    | 80-85 wt. % | Ta                    | ad 100 wt. % |
|    | 33.013      | Ti                    | 80-85 wt. % | Nb                    | ad 100 wt. % |
|    | 33.014      | Ti                    | 80-85 wt. % | W                     | ad 100 wt. % |
|    | 33.015      | Ti                    | 80-85 wt. % | Mo                    | ad 100 wt. % |
| 65 | 33.016      | Ti                    | 80-85 wt. % | Ta                    | ad 100 wt. % |
|    | 33.017      | Ti                    | 80-85 wt. % | Nb                    | ad 100 wt. % |
|    | 33.018      | Ti                    | 80-85 wt. % | W                     | ad 100 wt. % |
|    | 33.019      | Ti                    | 80-85 wt. % | Mo                    | ad 100 wt. % |

TABLE 33-continued

|        | Component 1 | Amount of component 1 | Component 2 | Amount of component 2 |
|--------|-------------|-----------------------|-------------|-----------------------|
| 33.012 | W           | 80-85 wt. %           | Ti          | ad 100 wt. %          |
| 33.013 | Mo          | 80-85 wt. %           | Ta          | ad 100 wt. %          |
| 33.014 | Mo          | 80-85 wt. %           | Nb          | ad 100 wt. %          |
| 33.015 | Mo          | 80-85 wt. %           | W           | ad 100 wt. %          |
| 33.016 | Mo          | 80-85 wt. %           | Ti          | ad 100 wt. %          |
| 33.017 | Ti          | 80-85 wt. %           | Ta          | ad 100 wt. %          |
| 33.018 | Ti          | 80-85 wt. %           | Nb          | ad 100 wt. %          |
| 33.019 | Ti          | 80-85 wt. %           | W           | ad 100 wt. %          |
| 33.020 | Ti          | 80-85 wt. %           | Mo          | ad 100 wt. %          |

Table 34: Table 34 consists of 20 alloys, pseudo alloys and powder mixtures according to Table 16, component 1 being present in an amount of 85-90 wt. %, component 2 being present in an amount ad 100 wt. % and the individual partners in the mixture being as listed in Table 16.

TABLE 34

|        | Component 1 | Amount of component 1 | Component 2 | Amount of component 2 |
|--------|-------------|-----------------------|-------------|-----------------------|
| 34.001 | Nb          | 85-90 wt. %           | Ta          | ad 100 wt. %          |
| 34.002 | Nb          | 85-90 wt. %           | W           | ad 100 wt. %          |
| 34.003 | Nb          | 85-90 wt. %           | Mo          | ad 100 wt. %          |
| 34.004 | Nb          | 85-90 wt. %           | Ti          | ad 100 wt. %          |
| 34.005 | Ta          | 85-90 wt. %           | Nb          | ad 100 wt. %          |
| 34.006 | Ta          | 85-90 wt. %           | W           | ad 100 wt. %          |
| 34.007 | Ta          | 85-90 wt. %           | Mo          | ad 100 wt. %          |
| 34.008 | Ta          | 85-90 wt. %           | Ti          | ad 100 wt. %          |
| 34.009 | W           | 85-90 wt. %           | Ta          | ad 100 wt. %          |
| 34.010 | W           | 85-90 wt. %           | Nb          | ad 100 wt. %          |
| 34.011 | W           | 85-90 wt. %           | Mo          | ad 100 wt. %          |
| 34.012 | W           | 85-90 wt. %           | Ti          | ad 100 wt. %          |
| 34.013 | Mo          | 85-90 wt. %           | Ta          | ad 100 wt. %          |
| 34.014 | Mo          | 85-90 wt. %           | Nb          | ad 100 wt. %          |
| 34.015 | Mo          | 85-90 wt. %           | W           | ad 100 wt. %          |
| 34.016 | Mo          | 85-90 wt. %           | Ti          | ad 100 wt. %          |
| 34.017 | Ti          | 85-90 wt. %           | Ta          | ad 100 wt. %          |
| 34.018 | Ti          | 85-90 wt. %           | Nb          | ad 100 wt. %          |
| 34.019 | Ti          | 85-90 wt. %           | W           | ad 100 wt. %          |
| 34.020 | Ti          | 85-90 wt. %           | Mo          | ad 100 wt. %          |

Table 35: Table 35 consists of 20 alloys, pseudo alloys and powder mixtures according to Table 16, component 1 being present in an amount of 90-95 wt. %, component 2 being present in an amount ad 100 wt. % and the individual partners in the mixture being as listed in Table 16.

TABLE 35

|        | Component 1 | Amount of component 1 | Component 2 | Amount of component 2 |
|--------|-------------|-----------------------|-------------|-----------------------|
| 35.001 | Nb          | 90-95 wt. %           | Ta          | ad 100 wt. %          |
| 35.002 | Nb          | 90-95 wt. %           | W           | ad 100 wt. %          |
| 35.003 | Nb          | 90-95 wt. %           | Mo          | ad 100 wt. %          |
| 35.004 | Nb          | 90-95 wt. %           | Ti          | ad 100 wt. %          |
| 35.005 | Ta          | 90-95 wt. %           | Nb          | ad 100 wt. %          |
| 35.006 | Ta          | 90-95 wt. %           | W           | ad 100 wt. %          |
| 35.007 | Ta          | 90-95 wt. %           | Mo          | ad 100 wt. %          |
| 35.008 | Ta          | 90-95 wt. %           | Ti          | ad 100 wt. %          |
| 35.009 | W           | 90-95 wt. %           | Ta          | ad 100 wt. %          |
| 35.010 | W           | 90-95 wt. %           | Nb          | ad 100 wt. %          |
| 35.011 | W           | 90-95 wt. %           | Mo          | ad 100 wt. %          |
| 35.012 | W           | 90-95 wt. %           | Ti          | ad 100 wt. %          |
| 35.013 | Mo          | 90-95 wt. %           | Ta          | ad 100 wt. %          |
| 35.014 | Mo          | 90-95 wt. %           | Nb          | ad 100 wt. %          |
| 35.015 | Mo          | 90-95 wt. %           | W           | ad 100 wt. %          |
| 35.016 | Mo          | 90-95 wt. %           | Ti          | ad 100 wt. %          |

TABLE 35-continued

|   | Component 1 | Amount of component 1 | Component 2 | Amount of component 2 |              |
|---|-------------|-----------------------|-------------|-----------------------|--------------|
| 5 | 35.017      | Ti                    | 90-95 wt. % | Ta                    | ad 100 wt. % |
|   | 35.018      | Ti                    | 90-95 wt. % | Nb                    | ad 100 wt. % |
|   | 35.019      | Ti                    | 90-95 wt. % | W                     | ad 100 wt. % |
|   | 35.020      | Ti                    | 90-95 wt. % | Mo                    | ad 100 wt. % |

10 Table 36: Table 36 consists of 20 alloys, pseudo alloys and powder mixtures according to Table 16, component 1 being present in an amount of 95-99 wt. %, component 2 being present in an amount ad 100 wt. % and the individual partners in the mixture being as listed in Table 16.

TABLE 36

|    | Component 1 | Amount of component 1 | Component 2 | Amount of component 2 |              |
|----|-------------|-----------------------|-------------|-----------------------|--------------|
| 20 | 36.001      | Nb                    | 95-99 wt. % | Ta                    | ad 100 wt. % |
|    | 36.002      | Nb                    | 95-99 wt. % | W                     | ad 100 wt. % |
|    | 36.003      | Nb                    | 95-99 wt. % | Mo                    | ad 100 wt. % |
|    | 36.004      | Nb                    | 95-99 wt. % | Ti                    | ad 100 wt. % |
|    | 36.005      | Ta                    | 95-99 wt. % | Nb                    | ad 100 wt. % |
|    | 36.006      | Ta                    | 95-99 wt. % | W                     | ad 100 wt. % |
|    | 36.007      | Ta                    | 95-99 wt. % | Mo                    | ad 100 wt. % |
|    | 36.008      | Ta                    | 95-99 wt. % | Ti                    | ad 100 wt. % |
|    | 36.009      | W                     | 95-99 wt. % | Ta                    | ad 100 wt. % |
|    | 36.010      | W                     | 95-99 wt. % | Nb                    | ad 100 wt. % |
|    | 36.011      | W                     | 95-99 wt. % | Mo                    | ad 100 wt. % |
|    | 36.012      | W                     | 95-99 wt. % | Ti                    | ad 100 wt. % |
|    | 36.013      | Mo                    | 95-99 wt. % | Ta                    | ad 100 wt. % |
|    | 36.014      | Mo                    | 95-99 wt. % | Nb                    | ad 100 wt. % |
|    | 36.015      | Mo                    | 95-99 wt. % | W                     | ad 100 wt. % |
|    | 36.016      | Mo                    | 95-99 wt. % | Ti                    | ad 100 wt. % |
|    | 36.017      | Ti                    | 95-99 wt. % | Ta                    | ad 100 wt. % |
|    | 36.018      | Ti                    | 95-99 wt. % | Nb                    | ad 100 wt. % |
|    | 36.019      | Ti                    | 95-99 wt. % | W                     | ad 100 wt. % |
|    | 36.020      | Ti                    | 95-99 wt. % | Mo                    | ad 100 wt. % |

## EXAMPLES

## Preparation of a Tantalum Powder

A tantalum hydride powder was mixed with 0.3 wt. % magnesium and placed in a vacuum oven. The oven was evacuated and filled with argon. The pressure was 860 Torr, a stream of argon was maintained. The oven temperature was raised to 650° C. in steps of 50° C. and, after a constant temperature had been established, was maintained for four hours. The oven temperature was then raised to 1000° C. in steps of 50° C. and, after a constant temperature had been established, was maintained for six hours. At the end of this time, the oven was switched off and cooled to room temperature under argon. Magnesium and the resulting compounds were removed in the conventional manner by acid washing. The resulting tantalum powder had a particle size of -100 mesh (<150 µm), an oxygen content of 77 ppm and a specific BET surface area of 255 cm<sup>2</sup>/g.

## Preparation of a Titanium Powder

The procedure was as for the preparation of the tantalum powder. A titanium powder having an oxygen content of 93 ppm was obtained.

## Preparation of a Pre-Alloyed Titanium/Tantalum Powder

A mixture of tantalum hydride powder and titanium hydride powder in a molar ratio of 1:1 was prepared and was mixed with 0.3 wt. % magnesium; the procedure as in the preparation of the tantalum powder was then followed. A titanium/tantalum powder having an oxygen content of 89 ppm was obtained.

## Production of Coatings

Tantalum and niobium coatings were produced. The tantalum powder used was AMPERIT® 150.090 and the niobium powder used was AMPERIT® 160.090, both of which are commercially available materials from H. C. Starck GmbH in Goslar. The commercially available nozzle of the MOC 29 type from CGT GmbH in Ampfing was used.

FIG. 7: Unetched cross-section of a tantalum coating, process gas nitrogen, overview picture with low magnification

FIG. 8: Unetched cross-section of a tantalum coating, process gas nitrogen

FIG. 9: Image section used for porosity determination, cross-section of a tantalum coating, process gas nitrogen

| Material                                                           | Tantalum                    | Tantalum                | Niobium            | Niobium            |
|--------------------------------------------------------------------|-----------------------------|-------------------------|--------------------|--------------------|
| Nozzle                                                             | MOC 29                      | MOC 29                  | MOC 29             | MOC 29             |
| Determination of the feed rate at 0.52 Nm <sup>3</sup> /h:         |                             |                         |                    |                    |
| 3.0 rpm (g/30 s/g/min)                                             | 35.5/71.0                   | 35.5/71.0               | 14.7/29.4          | 14.7/29.4          |
| 4.0 rpm (g/30 s/g/min)                                             |                             |                         | 19.8/39.6          | 19.8/39.6          |
| Movement data:                                                     |                             |                         |                    |                    |
| Spray speed/ speed of the nozzle over the substrate (m/min) (mm/s) | 20/333                      | 20/333                  | 20/333             | 20/333             |
| Line feed (mm)                                                     | 1.5                         | 1.5                     | 1.5                | 1.5                |
| Spraying interval (mm)                                             | 30                          | 30                      | 30                 | 30                 |
| Process gas:                                                       | Nitrogen                    | Helium                  | Nitrogen           | Helium             |
| Pressure (bar)                                                     | 30                          | 28                      | 30                 | 28                 |
| Flow (Nm <sup>3</sup> /h)                                          | 65                          | 190/He 181              | 60                 | 190/He 181         |
| Proportion of feed gas (%)                                         | 8                           | 3 (N2)                  | 8                  | 3 (N2)             |
| Powder feed                                                        |                             |                         |                    |                    |
| Powder feed rate (g/min)                                           | 71                          | 71                      | 39.6               | 39.6               |
| Number of passes                                                   | 3                           | 3                       | 3                  | 3                  |
| Substrates                                                         | 1FTa 1FS 1FV<br>1FS 1RV 1RS | 1FTa 1FV 2FS<br>1RV 1RS | 2FS 2FV 1RS<br>1RV | 2FS 2FV 1RV<br>1RS |
| Sheet thickness before (mm)                                        | 2.86                        | 2.92                    | 2.91               | 2.84               |
| Sheet thickness after (mm)                                         | 3.38                        | 3.44                    | 3.35               | 3.36               |
| Coating thickness, approx. (µm) *                                  | 520.00                      | 520.00                  | 436.00             | 524.00             |
| Porosity/Density                                                   | 0.9%/99.1%                  | 2.2%/97.8%              |                    |                    |

Substrates: The substrates were placed in succession on the specimen holder and coated under the indicated test conditions. The substrate description is made up as follows:

The number at the beginning indicates the number of identical substrates located next to one another. The following letter indicates whether a flat specimen (F) or a round specimen (R, tube) was used. The following letters indicate the material, Ta meaning tantalum, S meaning a structural steel, and V meaning a stainless steel (chromium-nickel steel).

Very strong and dense coatings were obtained, which exhibit low porosity and excellent adhesion to the substrates in question. The flow rate densities were between 11 and 21 g/sec\*cm<sup>2</sup>.

FIGS. 1 to 10 show light microscope pictures of cross-sections of the resulting tantalum coatings. No inclusions of copper or tungsten are detectable, as occurs with corresponding layers produced by vacuum plasma spraying. The porosity determination was carried out automatically by the image analysis program ImageAccess.

FIG. 1: Unetched cross-section of a tantalum coating, process gas helium

FIG. 2: Unetched cross-section of a tantalum coating, process gas helium, overview picture with low magnification

FIG. 3: Cross-section of a tantalum coating, etched with hydrofluoric acid, process gas helium, overview picture with low magnification

FIG. 4: Cross-section of a tantalum coating, etched with hydrofluoric acid, process gas helium

FIG. 5: Image section used for porosity determination, cross-section of a tantalum coating, process gas helium

FIG. 6: Cross-section of a tantalum coating, etched with hydrofluoric acid, interface with the substrate, process gas helium

35 FIG. 10: Unetched cross-section of a tantalum coating, process gas nitrogen, high magnification

The invention claimed is:

1. A method of applying coatings to a surface, the method comprising:

cold-spraying a gas flow at supersonic speed onto a surface of an object, thereby forming a coating on the surface, the gas flow comprising a mixture of gas with a powder of a bulk material selected from the group consisting of:

a) alloys, pseudo alloys, and powder mixtures of Nb, Ta, W, or Mo with

(i) each other, or with Ti or Zr, or

(ii) 2-30 wt. % of Co, Ni, Rh, Pd, Pt, Cu, Ag or Au; or

b) binary alloys, binary pseudo alloys, and binary powder mixtures of 2-50 wt. % Nb, Ta, W, or Mo with each other or with Ti or Zr,

wherein (i) the powder has a particle size of from 0.5 to 150 µm and an oxygen content of less than 1000 ppm, and (ii) the coating has a density of at least 97% of a density of the bulk material.

2. The method as claimed in claim 1, further comprising adding the powder to the gas in an amount such that a flow rate density of the particles of from 0.01 to 200 g/s cm<sup>2</sup>.

3. The method as claimed in claim 1, further comprising adding the powder to the gas in an amount such that a flow rate density of the particles of from 0.05 g/s cm<sup>2</sup> to 17 g/s cm<sup>2</sup>.

4. The method as claimed in claim 1, wherein the spraying comprises the steps of:

providing a spraying orifice adjacent the surface;

providing the powder to the spraying orifice under pressure;

providing the gas under pressure to the spraying orifice to establish a static pressure at the spraying orifice, thereby forming the gas flow, wherein the gas comprises an inert gas; and

locating the spraying orifice in a region of low ambient pressure which is less than 1 atmosphere and which is substantially less than the static pressure at the spraying orifice to provide substantial acceleration of the gas flow.

5. The method as claimed in claim 1, wherein the cold spraying is performed with a cold spray gun and the surface and the cold spray gun are located within a vacuum chamber at a pressure below 80 kPa.

6. The method as claimed in claim 1, wherein a speed of the powder in the gas flow is supersonic to 2000 m/s.

7. The method as claimed in claim 1, wherein the spraying is performed with a cold spray gun and the surface and the cold spray gun are located within a vacuum chamber at a pressure between 2 and 10 kPa and the speed of the powder in the gas flow is supersonic to 1200 m/s.

8. The method as claimed in claim 1, wherein the coating has a particle size of from 5 to 150  $\mu\text{m}$ .

9. The method as claimed in claim 1, wherein the powder has gaseous impurities of from 200 to 2500 ppm, based on weight.

10. The method as claimed in claim 1, wherein the coating has a particle size of from 10 to 50  $\mu\text{m}$  and the powder has an oxygen content of less than 500 ppm.

11. The method as claimed in claim 1, wherein the powder has an oxygen content of less than 100 ppm.

12. The method as claimed in claim 1, wherein the coating has an oxygen content of less than 1000 ppm.

13. The method as claimed in claim 1, wherein the coating has an oxygen content of less than 100 ppm.

14. The method as claimed in claim 1, wherein the coating has a content of gaseous impurities that differs by no more than 50% from a content of gaseous impurities of the powder.

15. The method as claimed in claim 1, wherein the coating has a content of gaseous impurities that differs by no more than 20% from a content of gaseous impurities of the powder.

16. The method as claimed in claim 1, wherein the coating has an oxygen content that differs by no more than 5% from an oxygen content of the powder.

17. The method as claimed in claim 1, wherein the coating has a content of gaseous impurities that differs by no more than 10% from a content of gaseous impurities of the powder.

18. The method as claimed in claim 1, wherein the coating has a content of gaseous impurities that differs by no more than 1% from a content of gaseous impurities of the powder

and wherein the coating has an oxygen content that differs by no more than 1% from an oxygen content of the starting powder.

19. The method as claimed in claim 1, wherein an oxygen content of the coating is no more than 100 ppm.

20. The method as claimed in claim 1, wherein a thickness of the coating is from 10  $\mu\text{m}$  to 10 mm.

21. The method as claimed in claim 1, wherein the powder is an alloy having from 94 to 99 wt. % molybdenum, from 1 to 6 wt. %, niobium, and from 0.05 to 1 wt. % zirconium.

22. The method as claimed in claim 1, wherein the powder is an alloy having from 95 to 97 wt. % molybdenum, from 2 to 4 wt. %, niobium, and from 0.05 to 0.02 wt. % zirconium.

23. The method as claimed in claim 1, wherein the powder is an alloy, pseudo alloy, or powder mixture of a refractory metal selected from the group consisting of niobium, tantalum, tungsten, and molybdenum with a metal selected from the group consisting of titanium, cobalt, nickel, rhodium, palladium, platinum, copper, silver, and gold.

24. The method as claimed in claim 1, wherein the powder consists essentially of a tungsten-rhenium alloy.

25. The method as claimed in claim 1, wherein the powder consists essentially of a mixture of a titanium powder with (i) a tungsten powder or (ii) a molybdenum powder.

26. The method as claimed in claim 1, wherein the powder comprises 2-30 wt. % of cobalt, nickel, rhodium, palladium, platinum, copper, silver, or gold.

27. The method as claimed in claim 1, wherein the powder comprises 2-50 wt. % of titanium.

28. A method of applying coatings to a surface, the method comprising:

30 cold-spraying a gas flow at supersonic speed onto a surface of an object, thereby forming a coating on the surface, the gas flow comprising a mixture of gas with a powder of a bulk material selected from the group consisting of:

a) alloys, pseudo alloys, and powder mixtures of Nb, Ta, W, or Mo with

(i) each other, or with Ti or Zr, or

(ii) 2-30 wt. % of Co, Ni, Rh, Pd, Pt, Cu, Ag or Au; or

b) binary alloys, binary pseudo alloys, and binary powder mixtures of 2-50 wt. % Nb, Ta, W, or Mo with each other or with Ti or Zr,

35 wherein (i) the powder has a particle size of from 0.5 to 150  $\mu\text{m}$  and an oxygen content of less than 1000 ppm, (ii) the coating has a density of at least 97% of a density of the bulk material, and (iii) cold-sprayed layers are formed/produced with deposition rates of more than 90%.

\* \* \* \* \*